



US007070847B2

(12) **United States Patent**  
**Efird et al.**

(10) **Patent No.:** **US 7,070,847 B2**  
(b4) **Date of Patent:** **\*Jul. 4, 2006**

(54) **ABRADED FABRICS EXHIBITING EXCELLENT HAND PROPERTIES AND SIMULTANEOUSLY HIGH FILL STRENGTH RETENTION**

(75) Inventors: **Scott W. Efird**, Moore, SC (US); **Louis Dischler**, Spartanburg, SC (US)

(73) Assignee: **Milliken & Company**, Spartanburg, SC (US)

(\*) Notice: Subject to any disclaimer, the term of this patent is extended or adjusted under 35 U.S.C. 154(b) by 0 days.

This patent is subject to a terminal disclaimer.

(21) Appl. No.: **10/235,342**

(22) Filed: **Sep. 5, 2002**

(65) **Prior Publication Data**

US 2003/0194938 A1 Oct. 16, 2003

**Related U.S. Application Data**

(63) Continuation-in-part of application No. 09/777,444, filed on Feb. 6, 2001, now abandoned, which is a continuation of application No. 09/569,473, filed on May 12, 2000, now Pat. No. 6,230,376, which is a continuation of application No. 09/252,513, filed on Feb. 18, 1999, now Pat. No. 6,112,381.

(60) Provisional application No. 60/317,548, filed on Sep. 5, 2001.

(51) **Int. Cl.**

**D06C 11/00** (2006.01)  
**B32B 33/00** (2006.01)

(52) **U.S. Cl.** ..... **428/91; 428/92**

(58) **Field of Classification Search** ..... **428/91, 428/92; 26/28, 29 R**  
See application file for complete search history.

(56) **References Cited**

**U.S. PATENT DOCUMENTS**

|               |         |                              |
|---------------|---------|------------------------------|
| 2,107,528 A   | 2/1938  | Feinberg                     |
| 2,277,937 A   | 3/1942  | Shryer                       |
| 2,896,304 A   | 7/1959  | Peroni                       |
| 2,926,414 A   | 3/1960  | Weiss et al.                 |
| 3,549,398 A   | 12/1970 | Watson                       |
| 3,650,800 A   | 3/1972  | Reiner                       |
| 3,731,352 A * | 5/1973  | Okamoto et al. ..... 28/112  |
| 3,894,318 A   | 7/1975  | Ito et al.                   |
| 3,899,810 A   | 8/1975  | Stanley et al. ..... 28/72.6 |
| 3,908,057 A   | 9/1975  | Smith, II ..... 428/151      |
| 3,973,359 A   | 8/1976  | Spencer et al.               |

|               |         |                               |
|---------------|---------|-------------------------------|
| 3,980,549 A   | 9/1976  | Grutza                        |
| 4,051,699 A   | 10/1977 | Carpenter, Jr. ..... 68/5     |
| 4,349,597 A   | 9/1982  | Fine et al. ..... 428/95      |
| 4,370,787 A   | 2/1983  | Feldkumper ..... 29/124       |
| 4,463,483 A   | 8/1984  | Holm                          |
| 4,468,844 A   | 9/1984  | Otto                          |
| 4,512,065 A   | 4/1985  | Otto                          |
| 4,607,409 A   | 8/1986  | Hishimura et al. ..... 8/152  |
| 4,608,128 A   | 8/1986  | Farmer et al.                 |
| 4,837,902 A   | 6/1989  | Dischler ..... 26/1           |
| 4,864,150 A   | 9/1989  | Mann et al. ..... 250/571     |
| 4,918,795 A   | 4/1990  | Dischler ..... 26/1           |
| 5,080,952 A * | 1/1992  | Willbanks ..... 428/91        |
| 5,199,957 A   | 4/1993  | Pascoe ..... 8/478            |
| 5,407,447 A   | 4/1995  | Teague et al. ..... 8/483     |
| 5,473,801 A   | 12/1995 | Straube et al.                |
| 5,505,739 A   | 4/1996  | Montesano                     |
| 5,617,902 A   | 4/1997  | Farley ..... 139/1            |
| 5,752,300 A   | 5/1998  | Dischler                      |
| 5,815,896 A   | 10/1998 | Dischler                      |
| 5,943,745 A   | 8/1999  | Dischler ..... 26/28          |
| 5,958,083 A   | 9/1999  | Onishi et al. ..... 8/102     |
| 6,015,707 A   | 1/2000  | Emalfarb et al. ..... 435/263 |
| 6,055,711 A   | 5/2000  | Weil et al. ..... 28/151      |
| 6,112,381 A   | 9/2000  | Dischler et al. ..... 26/28   |
| 6,230,376 B1  | 5/2001  | Dischler ..... 26/28          |
| 6,260,247 B1  | 7/2001  | Dischler et al. ..... 26/28   |
| 6,269,525 B1  | 8/2001  | Dischler et al. ..... 26/28   |
| 6,716,775 B1  | 4/2004  | Dischler et al. ..... 442/59  |

**FOREIGN PATENT DOCUMENTS**

|    |             |         |
|----|-------------|---------|
| GB | 2 328 957 A | 3/1999  |
| JP | 58-197366 A | 11/1983 |
| WO | 00 49217 A  | 8/2000  |

\* cited by examiner

*Primary Examiner*—Jenna-Leigh Befumo

(74) *Attorney, Agent, or Firm*—Terry T. Moyer

(57) **ABSTRACT**

The inventive method provides highly desirable hand to various different types of fabrics through the initial immobilization of individual fibers within target fabrics and subsequent treatment through abrasion, sanding, or napping of at least a portion of the target fabric. Such a procedure includes “nicking” the immobilized fibers thereby permitting the fibers to produce a substantially balanced strength of the target fabric in the fill and warp directions while also providing the same degree of hand improvements as obtained with previous methods. Furthermore, this process also provides the unexpected improvement of non-pilling to synthetic fibers as the “nicking” of the immobilized fibers results in the lack of unraveling of fibers and thus the near impossibility of such fibers balling together to form unwanted pills on the fabric surface. Fabrics treated by this process are also contemplated within this invention.

**8 Claims, 1 Drawing Sheet**



Fig. 1

## 1

**ABRADED FABRICS EXHIBITING  
EXCELLENT HAND PROPERTIES AND  
SIMULTANEOUSLY HIGH FILL STRENGTH  
RETENTION**

CROSS REFERENCE TO RELATED  
APPLICATIONS

This application is a continuation of Provisional Application Ser. No. 60/317,548, filed Sep. 5, 2001, which is a continuation-in-part of application Ser. No. 09/777,444, filed on Feb. 6, 2001 now abandoned, which is a continuation of application Ser. No. 09/569,473, filed on May 12, 2000, now U.S. Pat. No. 6,230,376, which is a continuation of application Ser. No. 09/252,513, filed Feb. 18, 1999, now U.S. Pat. No. 6,112,381. All of these parent, grandparent, and great-grandparent applications are herein entirely incorporated by reference.

FIELD OF THE INVENTION

The inventive method provides highly desirable hand to various different types of fabrics through the initial immobilization of individual fibers within target fabrics and subsequent treatment through abrasion, sanding, or napping of at least a portion of the target fabric. Such a procedure includes "nicking" the immobilized fibers thereby permitting the fibers to produce a substantially balanced strength of the target fabric in the fill and warp directions while also providing the same degree of hand improvements as obtained with previous methods. Furthermore, this process also provides the unexpected improvement of non-pilling to synthetic fibers as the "nicking" of the immobilized fibers results in the lack of unraveling of fibers and thus the near impossibility of such fibers balling together to form unwanted pills on the fabric surface. Fabrics treated by this process are also contemplated within this invention.

BACKGROUND

Materials such as fabrics are characterized by a wide variety of functional and aesthetic characteristics. Of those characteristics, a particularly important feature is fabric surface feel or "hand." The significance of a favorable hand in a fabric is described and explained in U.S. Pat. Nos. 4,918,795 and 4,837,902, both to Dischler, the teachings of which are both entirely incorporated herein by reference.

Favorable hand characteristics of a fabric are usually obtained upon conditioning of prepared textiles (i.e., fabrics which have been de-sized, bleached, mercerized, and dried). Prior methods of prepared-fabric conditioning have included roughening of the finished product with textured rolls or pads. It has now been discovered, surprisingly, that such conditioning would favorably be performed while the target fabric is in its greige state or is unprepared. The conditioning of such fabrics provides heretofore unknown benefits in improvements in overall fabric strength, and the like (as discussed in greater detail below). Of great importance and necessity then within the textile treatment industry is a procedure through which greige or unfinished fabrics can be treated and subsequently finished which provides desirable hand to the target textile and does not adversely impact the ability for dyeing, decorating, and the like, the textile at a future point in time. Such processes have not been taught nor fairly suggested within the pertinent art. Thus, there is no prior teaching nor fair suggestion within the pertinent art

## 2

which has accorded highly effective and easily duplicated textile hand improvements to greige goods and unfinished textiles.

In the textile industry, it is known to finish woven fabrics by abrading one or both surfaces of the fabric using sandpaper or a similarly abrasive material to cut and raise the fibers of the constituent yarns in the fabric. Through such a treatment, a resultant fabric is obtained generally exhibiting a closely raised nap producing a soft, smooth surface texture resembling suede leather. This operation, commonly referred to as suedeing or sanding, is conventionally performed by a specialized fabric suedeing machine wherein the fabric is passed under tension over one or more finishing rolls, covered with sandpaper or a similarly abrasive material, which are rotated at a differential speed relative to the moving fabric web. Such machines are described in U.S. Pat. No. 5,752,300 to Dischler, and U.S. Pat. No. 3,973,359 to Spencer, both hereby entirely incorporated by reference.

Another well known technique for enhancing aesthetic and performance characteristics of a fabric through the same type of surface-raising treatment is napping. Such a treatment provides a fabric exhibiting a softer hand, improved drapeability, greater fabric thickness, and better overall durability. Napping machinery generally utilizes rotatably driven cylinders including peripheral wire teeth, such as, normally, card clothing, over which the fabric travels under a certain amount of tension.

During a napping treatment the individual fibers are ideally pulled from the fabric body in contrast to suedeing which ideally cuts the individual fibers. Suedeing, however, presents some disadvantages including the fact that a certain amount of napping occurs simultaneously. Grit particles engage the surface fibers of the target fabric and inevitably pull them from the fabric body resulting in a relatively long pile. Such a long pile traps air at the surface of the fabric creating an insulating-type effect which thereby produces a warm feeling against the wearer's skin. Such an insulating effect is highly undesirable, particularly for apparel intended for summer wear. Upon utilization of strong synthetic fibers (i.e., nylon or polyester), this tendency for fibers to be pulled from the surface of the fabric is accentuated. More tension would thus be required to cut through such strong fibers (as compared to the force necessary to cut weaker ones) and the stronger fibers then are pulled more easily from the yarn. Upon engagement by an abrasive grit particle, sufficient tension to pull rather than easily cut the fibers is accorded. Pilling is thus more noticeable with strong synthetic fibers and where a long pile is created (and thus highly disadvantageous) because entanglement between adjacent fibers is more likely to occur, thereby resulting in highly objectionable and unwanted pills on the fabric surface.

Methods have been utilized in the past on prepared fabrics to produce a short pile in order to decrease the potential for pilling. These have included the use of sand paper with very fine grit, brush rolls with grit particles embedded in soft nylon bristles, and even blocks of pumice stone mounted upon oscillating bars. However, the fine grit sandpaper degrades easily and rapidly due to the loss of grit particles and the build-up of debris between the remaining particles. Furthermore, the target fibers are not cut in this fashion as much as they are generally eroded. Thus, fine grit sandpaper does not provide an effective process of replacing the suedeing techniques mentioned above. Soft nylon bristles also appear to merely erode the fibers away than cut and also is highly inefficient because of the light pressure such devices apply to the target fabric. Pumice stone, being very soft, is itself subject to damage in such operations and also

facilitates unwanted build-up of fibrous debris within the treatment surface of the stone. Undesirable wet procedures are generally necessary to produce any effective sueding results for pumice stone and fine grit sandpaper treatments.

Another disadvantage of prior napping and/or sueding treatments concerns the situation where fill yarns are exposed on the surface of the target fabric. Being perpendicular to the action of the napping and/or sueding, such treatments tend to act primarily upon these exposed yarns rather than the warp yarns. Weaving economy generally dictates that the target fabric would be more heavily constructed in the warp direction and thus it would be highly advantageous for sueding to act primarily on such warp yarns since those yarns exhibit more strength to relinquish during the abrasion procedure.

As noted above, one of the most unpleasant and unsightly phenomena produced through the utilization of strong synthetic fibers within fabrics is pilling. This term is generally accepted to mean the formation of small balls of fiber which are created on the textile surface by the entanglement of free fiber ends. Such fibers which hold the pills to the base fabric do not break off because the synthetic fibers (such as polyester) exhibit a higher flex strength than natural fibers and thus small balls of twisted and entangled fiber cling to the fabric surface.

A number of procedures have been developed to counter this undesirable pilling effect within the textile industry. For instance, polyester fibers have been produced with low molecular weights or low solution viscosities in order to reduce the strength of the fibers resulting in fiber ends and nascent pills which more readily break off from the fabric surface (oust as with natural fibers). However, such a reduction in strength (by about 40% from standard polyester fibers) leaves them highly susceptible to damage during further processing thus prohibiting processing on ring or rotor-spinning frames at the same speeds and with the same efficiencies as normal types of natural fibers (such as cotton). A further method to control pilling concerns the chemical weakening of fibers within woven fabrics. This is accomplished through the application of super-heated steam or aqueous solutions of acids, ammonia, ammonia vapors, or amines. In such an instance, however, the entire fabric strength is sacrificed with no concomitant enhancement of hand. Furthermore, the potential for fabric defects (such as stains and uneven dyeing) is increased. An additional method is to utilize yarns having high twist. However, such resultant fabrics exhibit a harsh hand and the internal compression generated by the twist of the individual fibers makes it very difficult to properly de-size, mercerize, and dye fabrics comprising such high-twist yarns. It would thus be highly desirable to obtain substantial reduction in pilling for fabrics comprising strong synthetic fibers without recourse to the above processes and methods. Unfortunately, the prior art has not accorded such an improvement with a simultaneous improvement in hand of the fabric.

The present invention provides a hand improvement method to unfinished fabrics in a manner not disclosed in the known prior art. Such a method also substantially eliminates pilling in fabrics comprised of synthetic fibers simultaneously while providing the aforementioned improvements of the hand of the target fabric.

#### BRIEF DESCRIPTION OF THE DRAWING

FIG. 1 is a side schematic view of an apparatus useful in performing the instant invention, illustrating one manner in which a fabric may be processed according to the invention.

#### DESCRIPTION

The primary object of this invention is therefore to provide improved sueded hand to greige or unprepared fabrics while also retaining a balanced strength over the entire fabric structure. It is thus an additional advantage of this invention to provide such a method that is highly cost-effective and enhances subsequent fabric processing such as de-sizing, mercerization, dyeing, and the like.

10 Another object of this invention to be provide a method of improving the hand of unfinished fabrics comprising synthetic fibers which simultaneously substantially eliminates pilling on the fabric surface. Yet another advantage of this invention is to provide a sueded cotton/polyester blended fabric wherein the sueded surface is dominated by relatively soft polyester fibers. These and other advantages will be in part apparent and in part pointed out below.

In order to improve the hand of fabrics in a manner which is consistent with warm weather wear, the constituent fibers 20 must be treated in a manner which provides a consistently short pile, so that a stagnant layer of insulating air is not trapped at the fabric surface. It has been found that, by first immobilizing the fibers constituting the fabric with a temporary coating, followed by an abrasive treatment of the 25 fabric surface, and then removal of the temporary coating, a fabric of unique aesthetic and practical characteristics is obtained. Compared to a fabric which has been sanded or napped, a fabric treated by the present inventive method is cooler to the touch, smoother to the hand, and dramatically 30 more resistant to pilling. To understand how these advantageous characteristics are obtained, it is useful to compare the action of card wire on a film of polyester (e.g., Mylar® film) to the action of the wire on a polyester fabric. When card wire is dragged across a Mylar® film under pressure, many 35 small scratches are seen to develop in the surface, due to the combination of high pressure at the wire tip combined with the high hardness of the wire relative to polyester. When the wire is similarly dragged across the polyester fabric, scratches are generally not found since the motion of the 40 fibers relative to each other allows the stresses to be dissipated before abrasive wear occurs. Also, the interaction of wire and fiber typically tensions the fiber and draws it away from the yarn surface. When the fabric assumes the characteristics of a film, scratching of the fiber surface does then 45 occur, and pulling out of fibers from the yarn is prevented. Thus, the fabric is transformed into film (or composite), abraded, and then transformed back into a fabric. What would be linear scratches on a film appear as nicks of various sizes on the surface fibers, including nicks which 50 entirely cut through some of the fibers. The cut fiber ends will be released during subsequent processing (e.g., de-sizing) to form a pile which is uniformly short. Short fibers resist forming pills because the number of adjacent fibers available for entanglement is limited to those few within 55 reach of each other. "Nicks" on these fibers serve as stress risers, allowing the fiber to break off during the kind of bending that occurs during pill formation. Since only the surface fibers have been so weakened, the bulk of the fabric strength has been retained as compared to chemical treatments, which necessarily weaken the entire fabric structure.

The term "nicking" basically encompasses the creation of cuts at random locations on individual fibers thus providing stress risers on the individual fibers. The immobilization of these fibers thus increases frictional contact between the individual fibers and prevents movement of the fibers during the sanding, abrading, or napping procedure. The abrading, sanding, or napping of non-immobilized fibers which move

during treatment can result in the relative motion of the fibers and the pulling out of long fibers as the fibers interact with the abrasive or napping media. Such a process does provide improvements in the hand of such fabrics; however, the filling strength of the fabric may be sacrificed and the ability of the fabric to trap unwanted air (thus producing a "warmer" fabric) is increased. Therefore, the inventive process comprises first immobilizing the surface fibers of a fabric with a temporary coating; second, treating the immobilized surface fibers by abrasion, sanding, or napping in order to cut and "nick" the fibers; and third, removing, in some manner, the temporary coating.

The immobilization step thus comprises encapsulating at least the surface fibers (and possibly some of the internal fibers of the fabric) in a coating matrix which makes the fibers stationary to the point that the individual fibers are resistant to motion due to the space-filling characteristics of the coating matrix within the interstices between the fibers, as well as the adhesion of adjacent fibers by the coating matrix. A typical coating matrix which imparts immobilization on the surface fibers of a target fabric is size (i.e., starch, polyvinyl alcohol, polyacrylic acid, and the like) which can easily be removed through exposure to water or other type of solvent. Usually, size is added to warp yarns prior to weaving. In accordance with this invention, the size already present in the greige goods to be abraded may be employed for the purpose of immobilization; alternatively, additional size may be coated onto the target fabric to provide a sufficient degree of rigidity.

To be effective (i.e., to impart the proper degree of rigidity or immobilization to the target fibers), the coating does not have to fill the entire free space of the yarn; however, a solids coating level of between 5 and 50% by the weight of the fabric has been found to be particularly effective. A coating range of between 10 and 25% of the weight of the fabric is most preferred. In one particularly preferred embodiment, a greige fabric is to be subsequently treated through sanding, abrading, or napping but does not require any further application of size. As long as the size present during the weaving procedure is not removed thereafter, sufficient rigidity will exist for proper immobilization of the target fabric for further treatment by sanding, abrading, or napping within the inventive process. Another preferred method of immobilization through size application is to dissolve the coating agent in water and pad onto the fabric, followed by a drying step; however, this encompasses both sized (greige) and de-sized fabrics.

Another temporary coating available within the inventive immobilization step is ice. In such an instance, 50 to 200% by weight of water is applied to the target fabric that is subsequently exposed to subfreezing temperatures until frozen. The fabric is then abraded while frozen and then dried. One embodiment of this type of immobilization includes padding on at least about 50% of the fabric and at most about 200% of the water and then freezing the fabric in situ. Such a method may be utilized on greige, prepared, or finished goods and it eliminates the need to add extra amounts of size to an already-woven fabric. This elimination of the need to add and recover size is therefore highly cost-effective. If ice is utilized to immobilize the constituent fibers of the target fabric, napping with metal wires or brushes is the preferable method of treating the target fabric. Wire allows ice, which has melted and refrozen, to break free easily. The resultant ice film could render sanders and/or abraders ineffective since the grit generally utilized in those procedures is very small and would not penetrate through the film to "nick" the individual fibers as is necessary for this inventive process to

function properly. The frozen target fabric is preferably maintained at a low temperature (at least from about -10 to about -50° C.), both to insure that the ice has sufficient shear strength for immobilization, and to provide enough heat capacity to absorb the mechanical energy imparted by the abrasion process without melting.

As noted above, the size employed as an aid to weaving may be retained subsequent to weaving, and employed in the present invention to immobilize the target fibers. This is believed to be unique within the textile industry. While such processes as singeing and heat-setting may be applied to greige goods, neither process obtains the advantages from the presence of size on the greige fabric. Otherwise, size is removed from greige goods prior to any further treatment (such as mercerizing, bleaching, dyeing, napping, sanding, and the like).

The most important step to the inventive method is the immobilization of the surface fibers. Thus, abrading, sanding, napping, and the like, may be utilized within the inventive process. Thus, abrading through contacting a fabric surface with an abrasive-coated cylindrical drum rotating a speed different from that of the fabric web is one preferred embodiment within this inventive process. Such a method is more fully described in U.S. Pat. Nos. 5,752,300 and 5,815,896, both to Dischler, herein entirely incorporated by reference. Angular sueding, as in U.S. patent application Ser. No. 09/045,094 to Dischler, now U.S. Pat. No. 5,943,745, also herein entirely incorporated by reference, is also an available method. The preferred abrasive is diamond grit embedded in an electroplated metal matrix that preferably comprises nickel or chromium, such as taught within U.S. Pat. No. 4,608,128 to Farmer. Other hard abrasive particles may also be used such as carbides, borides, and nitrides of metals and/or silicon, and hard compounds comprising carbon and nitrogen. Electroless plating methods may also be utilized to embed diamond and other hard abrasive grit particles within a suitable matrix. Preferably, the diamond grit particles are embedded within the plated metal surface of a treatment roll with which the target fabric may be brought into contact so that there is motion of the fabric relative to the grit particles. Since both the diamond facets and the metal matrix are microscopically smooth, build-up of size coating on the abrasive treatment surface is generally easily avoided. However, as noted previously, a more severe problem occurs where ice is utilized as the immobilizing matrix. The pressure of the fabric in contact with the small abrasive grit particles may cause the ice to melt and instantly refreeze onto the abrasive-coated cylinder. Also, since ice is generally weaker than polymeric sizing agents, a greater weight add-on is required to provide sufficient rigidity to the individual fibers. A thicker layer of coating thus results on the surface, and this superficial ice thickness interferes with the contact of the grit particles with the target fibers. As such, the grit particles would not be sufficient to "nick" the surface fibers. In such an instance, a napping procedure is preferred which utilizes wire brushes to condition the fabric surface, as taught in U.S. Pat. No. 4,463,483 to Holm. A cylindrical drum may still be utilized in such a situation with a napping wire wrapped around the drum which is then brought into contact with the target fabric, again a speed different from that of the fabric web. Normally, napping in this manner pulls the surface fibers away from the fabric surface; in the inventive method, the fibers are held in place and the desirable and necessary "nicking" of the individual fibers is thus accomplished. The bending of the wire during contact with the fabric allows ice to continually break free while the

length of the wire insures that the ice coating can be penetrated and the "nicking" procedure is, again, accomplished.

The particular types of fabrics which may be subjected to the inventive method are myriad. Such include, without limitation, any synthetic and/or natural fibers, including synthetic fibers selected from the group consisting of polyester, polyamide, polyaramid, rayon, lycra, and blends thereof, and natural fibers are selected from the group consisting of cotton, wool, flax, silk, ramie, and any blends thereof. The fabrics may also be constructed as woven, non-woven, and/or knit materials. Preferably, the target fabric comprises synthetic fibers and is woven. More preferably, the fabric comprises woven polyester fibers in spun yarns.

It has been determined that warp-faced twill fabrics are particularly suited to this inventive process because all of the exposed surface yarns of the woven substrate are sized which thus results in immobilization of all of the desired fibers thereby facilitating the "nicking" procedure described above. Furthermore, the costs associated with padding on size, drying, and de-sizing may also be avoided in some cases by abrading the fabric in the greige state. Usually, the warp yarns are sized prior to weaving in order to protect them from damage while fill yarns are generally untreated. If the fabric is warp-faced (e.g., a warp-faced twill fabric), then the abrasion step may be directly performed on the face, without any added processing steps required. Surprisingly, this approach has been found to be successful with plain woven fabrics, even though the fill yarns are not sized. In these fabrics, directly from the loom, the fill is comparatively straight and therefore is buried in the fabric structure (and thus much less accessible to the abrasive treatment). Generally, fabric that has been so treated is then processed in the normal manner, which typically combines steps such as de-sizing, mercerizing, bleaching, dyeing, and finishing. In special cases, the fabric may be sold to converters directly after the abrasion process. The converter would then do all or part of the subsequent processing. In cases where the size has functionality, it can be left on the fabric and can become part of the final product. For instance, in the case of abrasive-coated cloth (i.e., where it is desired to bond abrasive grit particles to the cloth) the size acts as a primer coat keeping the resin at the surface and physically preventing it from penetrating the body of the cloth in an uncontrolled fashion.

Also of particular interest within this invention is the fact that sueding of cotton/synthetic fiber blend fabrics in the greige state, prior to mercerization, is now known to produce unexpectedly beneficial effects. Historically, synthetic fibers for use in apparel, including polyester fibers, have generally been supplied to the textile industry with the object of duplicating or improving upon the characteristics of natural fibers. Such synthetic textile filaments were mostly of deniers per filament (dpf) in a range similar to those of the standard natural fibers (i.e., cotton and wool). More recently, however, polyester filaments have been available on a commercial level in a range of dpf similar to natural silk (i.e., of the order of 1 dpf), and even in subdeniers (below 1 dpf). Such fibers are considerably finer and more flexible than typical cotton fibers and thus are potentially preferred in the industry over such natural fibers. It has thus been discovered that fabrics containing cotton blended with such low dpf polyester fibers treated in accordance with this inventive method, then subsequently mercerized, exhibit a sueded surface that is substantially dominated by the synthetic fibers. This effect occurs because the cotton portion of

the generated pile tends to kink, bend, and shorten due to the swelling effect of the caustic on the cut cotton fibers. These fibers tend to swell to the greatest possible degree since they are not tensioned. Kinking and bending is further accentuated by the presence of "nicks" on these fibers, resulting in localized swelling where the cuticle of the cotton fiber is breached. The same effect does not occur with the cut polyester or other synthetic fibers that do not swell in the presence of caustic, so that the synthetic fibers ultimately dominate the surface aesthetics. This is advantageous when the target fabric contains synthetic fibers that are more flexible than mercerized cotton fibers, usually in the range of 1.5 dpf or less for polyester fibers. Such a benefit has not been readily available to the industry until now.

The above as well as other objects of the invention will become more apparent from the following detailed examples representing the preferred embodiments of the invention. A preferred method for abrading the fabric surface is illustrated in FIG. 1; except where otherwise stated, this machine set up was used to produce the fabrics described in the examples. The fabric F was fed to the abrasive rolls in a face-up configuration at an initial LPT tension at R1 of 110 lbs and a speed of 120 yards per minute. The fabric F was treated on its face in Section A by treatment rolls A1, A2, A3 and A4. The LEN measure tension at R2 was 72±15 lbs. The abrasive rolls A1, A2, A3, A4, B1, B2, B3 and B4 were 400 grit diamond plated rolls of the variety described previously. The abrasive rolls were turned in a clockwise or counterclockwise direction at a designated percentage of machine speed. A1 rotated counterclockwise at 400% speed, A2 rotated clockwise at 200% machine speed, A3 rotated counterclockwise at 400% machine speed, A4 rotated clockwise at 200% speed. The back of the fabric was treated in Section B. B1 rotated clockwise at 400% speed, B2 rotated counterclockwise at 200% speed, B3 rotated clockwise at 400% speed, and B4 rotated counterclockwise at 200% line speed. Relative to the speed of the fabric, each roll was running 300%, which gave an even treatment with and against the fabric. The tension at R3 was 300+20 lbs (critical measure setpoint), at LCN measured tension at R4 was 195±30 lbs, and at R5 was 165+20 lbs (critical measure setpoint.)

#### EXAMPLE 1

Four samples of 7.5 ounce per linear yard (66 inches wide) warp-faced twill fabric comprised of an intimate blend of 65% polyester and 35% cotton and completely constructed of open-end spun yarns were treated. One was a prepared fabric (i.e., already de-sized, bleached, mercerized, and dried) subjected to sanding alone and the other three were of the same fabric style prior to preparation. The combined level of abrasion for the front and back of all four test fabrics was the same, with varying proportions of such individual front and back sanding performed. The four samples, along with an untreated control, were then dyed, finished, and ultimately subjected to 10 industrial washes prior to testing.

The sanding operation was performed through contact with two pairs of 4.5" diameter rolls equipped with 320 U.S. grit diamonds in an electroplated nickel matrix. Each side of the fabric was treated by one pair of rolls (unless noted below to the contrary). The first roll for each side rotated against the direction of fabric travel and the second rotated with the fabric travel direction. The fabric subjected to the inventive procedure was a greige fabric, the fibers of which

were already sufficiently immobilized through the presence of the size (polyvinyl alcohol) applied to the constituent warp yarns prior to weaving.

Strength performance was analyzed through measurements of the tensile strength of the fabrics in different directions. The tensile strengths (pounds per inch to break) were measured in both the warp and fill directions. The warp/fill ratio, as used below, is the ratio of the warp to fill tensile strengths. For a fabric with balanced overall tensile strength, this ratio would be 1.0. Abrading a fabric so that the warp/fill ratio is close to 1.0 is the ideal, as it results in an isotropic material with no weak direction, and makes the most efficient use of the starting tensile strengths of the fabric. Pilling performance was measured through an empirical analysis and rating system. Such ratings ran from 1 (worst) to 5 (best), with such lower numbers indicating a high degree of undesirable pilling on the surface and a higher number denoting the lack of appreciable amounts of pills on the test fabric surface.

The five samples were tested (3 subjected to the inventive procedure, one as a sanded control, and the remaining sample unsanded). Run #1 involved the greige fabric with retained size treated through a sanding procedure which constituted equal abrasion between the face and the back of the target fabric (50% face/50% back). Run #2 was also subjected to the inventive process and constituted a 60% face/40% back sanding procedure. Run #3 involved a 100% face sanding procedure within the inventive process. Run #4 treated a control sample by a 50%/50% sanding procedure, and Run #5 was a control sample which was not treated by sanding at all (and thus exhibited a harsh hand and other undesirable characteristics for apparel uses). The results of these analyses are provided below in tabulated form:

TABLE

| Run        | Fabric Strength |              |           |  | Pilling Rating |
|------------|-----------------|--------------|-----------|--|----------------|
|            | Warp Tensile    | Fill Tensile | Warp/Fill |  |                |
| 1          | 148             | 115          | 1.29      |  | 4.5            |
| 2          | 135             | 130          | 1.04      |  | 4.5            |
| 3          | 148             | 139          | 1.06      |  | 4.5            |
| 4(Control) | 146             | 93           | 1.57      |  | 4.0            |
| 5(Control) | 176             | 138          | 1.28      |  | 4.0            |

Clearly, the prepared (control) fabrics exhibit unbalanced tensile properties with the warp about 28% stronger than the fill. Sanding both sides of these fabrics increases this imbalance to 57%, while the fabrics subjected to the inventive processes exhibited an average reduction in fabric direction strength imbalances. Since the strength of the fabric as a whole is governed by the fabrics' weakest direction, the greatest sueding efficiency is realized when the warp and the fill have similar final strengths as was achieved and best evidenced through following the inventive process.

## EXAMPLE 2

Two samples, one subjected to the inventive process and the other a control, of 4.8 ounces per square yard warp-faced twill comprised of an intimate blend of 65% polyester/35% cotton open-end spun yarns were treated in the same manner as in Run #s 1 and 5 of EXAMPLE 1, above. After 10

industrial washes, the control fabric exhibited a pilling rating of 2.0 while the fabric subjected to the inventive process showed a pilling rating of 4.0.

## EXAMPLE 3

Two samples, one subjected to the inventive process and the other a control, of 5.2 ounces per square yard plain woven fabric comprised of open-end spun polyester yarns were treated in accordance with Run #s 1 and 5 of EXAMPLE 1, above, with the following variation. As both samples were prepared fabrics (i.e., they did not contain size), a solution of 15% PVA size was dissolved in water and padded on to the inventive process fabric for a wet pick-up of 100%. After drying at 135° C. for 15 minutes, this fabric was then sanded on both sides (50% face/50% back). Both samples were then washed and heat-set. The samples treated in accordance with the inventive process was found to exhibit about a 5.0 pill rating. The heat-set control sample, to the contrary, exhibited a very high degree of pilling for a 1.0 rating.

## EXAMPLE 4

The same type of plain woven fabric as in EXAMPLE 3 was wet out with water so that the weight of the fabric approximately doubled. The wet fabric was then placed on a stainless steel cold plate for which the temperature was maintained between about -20 and -50° C. through contact with dry ice directly below the plate. Upon complete freezing of the water, the fabric face was scrubbed in the warp direction with straight carding wire. After this abrasion procedure, the fabric was dried to remove all moisture. A very short and even pile was developed which exhibited substantially no pilling for a rating of 5.0.

## EXAMPLE 5

Again, the same type of plain woven fabric as in EXAMPLE 3 was utilized but this time a continuous web of the fabric was wet out and passed into a bath of liquid nitrogen. The face of the frozen fabric was then abraded by contact with rotating rolls having axes oriented in the fill direction of the fabric web and wrapped with straight carding wire. The first roll turned in the direction opposite of fabric travel and the second turned with the fabric travel direction. Upon heating and drying, the fabric exhibited a very short and even pile and was found to have substantially no pills for a rating of 5.0. An untreated plain woven fabric control fabric, on the other hand, exhibited a high degree of pilling for a rating of 1.0.

## EXAMPLE 6

A 4.35 oz/sq yd fabric was woven in a plain weave construction using 26/1 OE 65/35 polyester/cotton yarns in the warp and 26/1 OE 65/35 polyester/cotton yarns in the filling. The woven fabric had approximately 103 ends per inch and 50 picks per inch. A sample of the fabric was retained in its unsanded form as Ex. 6A, while another sample was sanded in a conventional manner as follows: The fabric was processed on a machine of the variety described

## 11

in commonly-assigned U.S. Pat. No. 5,752,300 to Dischler. The fabric was processed using two rolls against the face and two against the face and two against the fabric back, with one of each of the pairs of rolls turning with the fabric and the other turning in a direction opposite that in which the fabric was moving. Three hundred pounds of tension were applied to the fabric, the fabric was processed at 120 yards per minute, and the rolls were turning at a speed of approximately 4 yards per minute. The rolls used were 300 grit rolls. For the sake of clarity, this sample will be referred to as Ex. 6B.

Another sample of the fabric was then face finished using a process according to the instant invention as follows: The fabric was processed in its greige form on a machine of the variety illustrated in FIG. 1 of U.S. Pat. No. 6,233,795 using the roll set up described in Attachment A, specifically, the fabric was treated sequentially on its face by a series of 400 grit rolls comprising a first roller running counter clockwise at 400% of machine speed, a second roller running clockwise at 200% machine speed, a third roll running counter clockwise at 400% of machine speed, a fourth roll running clockwise at 200% machine speed. The back of the fabric was likewise treated sequentially by a fifth roll running clockwise at 400% machine speed, a sixth roll running counter clockwise at 200% machine speed, a seventh roll running clockwise at 200% machine speed. (It is to be noted that the rolls that acted on the back of the fabric were parallel to the rolls that treated the front side of the fabric, so that that the fabric traveled in a U-shaped path. The machine speed was 120 yards per minute, and the result was an evenly treated fabric with unique hand and strength characteristics. The fabric was then prepared via a conventional desizing and scouring process, and a conventional chemical finish designed to enhance the fabric's soil release characteristics was applied. (The application of such chemistry is known to those of ordinary skill in the art, and is not described herein further in that is not believed to be essential to the invention.) The fabric was then exposed to high pressure hot air using a device of the variety described in commonly-assigned U.S. Pat. Nos. 4,837,902 and 4,918,795 to Dischler, the disclosures of which are incorporated herein by reference. The fabrics were then sanforized in a conventional manner, as will be readily understood by those of ordinary skill in the art. The fabric for the sake of clarity is referred to as Ex. 6C.

Each of the samples was then tested for strength in the filling direction according to ASTM D1682 (current method). The results are listed below.

## EXAMPLE 7

A 7.0 oz/sq yd fabric was woven in a 2x1 twill weave construction using 16/1 OE 65/35 polyester/cotton yarns in the warp and 12/1 OE 65/35 polyester/cotton yarns in the filling. The woven fabric had approximately 88 ends per inch and 46 picks per inch. A sample of the fabric was retained in its unsanded form (Ex. 7A), while another sample was sanded in the conventional manner as described above in Sample 6B, although in this case the fabric was processed at 80 yards per minute, at 400 pounds of tension. (This sample is Ex. 7B.) Another sample of the fabric was

## 12

then face finished using the same process of the instant invention described above in Example 6C (to form Ex. 7C). Each of the samples was then tested for strength in the filling in the manner of Example 6. The results are listed below.

## EXAMPLE 8

A 5.0 oz/sq yd fabric was woven in a plain weave construction using 26/1 OE spun 65/35 polyester/cotton yarns in the warp and 20.5/1 OE 65/35 polyester/cotton yarns in the filling. The woven fabric had approximately 102 ends per inch and 52 picks per inch. A sample of the fabric was retained in its unsanded form, while another sample was sanded in the conventional manner as described above in Example 6B. Another sample of the fabric was then face finished using the same process of the instant invention described above in Example 6C. Each of the samples was then tested for strength in the filling direction in the manner of Ex. 6. The results are listed below (Exs. 8A, 8B, and 8C, respectively).

## EXAMPLE 9

A 4.5 oz/sq yd fabric of the variety that would typically be used in top weight apparel was woven in a plain weave construction using 19/1 OE 100% polyester yarns in the warp and 26/1 OE 100% polyester yarns in the filling. The finished construction had approximately 80 ends per inch by 48 picks per inch. This fabric was sanded in the conventional manner described above in Example 6B. For purposes of clarity, the fabric processed in this manner is identified as 9A herein. The fabric was also processed according to the instant invention, as described in Ex. 6C (Ex. 9B).

A commercially available sanded 100% spun polyester fabric of the same weight and weave construction of those of 9A and 9B was obtained. The fabric was subjected to the same tests as 9A and 9B (described further below) in order that the fabric of the invention could be compared to another sanded fabric marketed for the same types of end uses. For purposes of identification, that fabric will be referred to as 9C herein.

## EXAMPLE 10

A 7.25 oz/sq yd fabric of the variety that would typically be used in bottom weight apparel was woven in a 2x1 twill weave construction using 12/1 OE 100% polyester yarns in the warp and 12/1 OE 100% polyester yarns in the filling. The finished construction had approximately 64 ends per inch by 50 picks per inch. This fabric was processed in the conventional manner described above in Ex. 6B. For purposes of clarity, the fabric processed in this manner is identified as 10A herein.

The fabric was also processed according to the instant invention, in the manner of 6C, to produce Example 10B.

A commercially available sanded 100% spun polyester fabric of the same weight and weave construction as those of 10A and 10B was obtained. That fabric was subjected to the same tests as 10A and 10B in order that the fabric of the invention could be compared to another sanded fabric marketed for the same types of end uses. For purposes of identification, that fabric will be referred to as 10C herein.

Percentages of retained filling strength were calculated for each of Examples 6–10 dividing the filling strength of the treated fabric by unsanded filling strength. The results for each are listed in the table below.

TABLE A

| Example | Filling Strength of Unsanded | Filling Strength of Conventionally Treated | Filling Strength When Processed According to the Invention | % Filling Strength Retained of Conventionally Treated | % Filling Strength Retained When Processed According to the Invention |
|---------|------------------------------|--------------------------------------------|------------------------------------------------------------|-------------------------------------------------------|-----------------------------------------------------------------------|
| Ex. 6   | 60 lbs                       | 52 lbs                                     | 59 lbs                                                     | 86.67%                                                | 98.33%                                                                |
| Ex. 7   | 120 lbs                      | 101 lbs                                    | 114 lbs                                                    | 84.17%                                                | 95.00%                                                                |
| Ex. 8   | 79                           | 69                                         | 75                                                         | 87.34                                                 | 94.94%                                                                |
| Ex. 9   | 87                           | 62                                         | 82                                                         | 71.26                                                 | 94.25%                                                                |
| Ex. 10  | 177                          | 132                                        | 180                                                        | 74.58                                                 | 101.69%                                                               |

As illustrated, the fabric of the invention retain at least about 85%, more preferably at least about 90%, even more preferably at least about 93%, even more preferably at least about 95%, and even more preferably at least about 98% or even at least about 100% of its fill strength. In a particularly preferred form of the invention, the fabric retains substantially all of its original filling strength. As will be readily appreciated by those of ordinary skill in the art, the filling is generally where most woven fabrics initially fail. Therefore, manufacturers must be cautious when face finishing fabrics in an attempt to improve their hand to keep from lowering the strength of the fabric to an extent that the durability of the fabric is impacted to great of an extent. Because the fabrics of the invention keep a significant portion of their initial strength, and in particular, the strength in the filling direction, the fabric retains a desirable level of strength and durability. Also, the fabrics of the invention have desirable hand characteristics.

The fabrics of Examples 9 and 10 were all tested to determine the following characteristics using the Kawabata Evaluation System ("Kawabata System"). The Kawabata System was developed by Dr. Sueo Kawabata, Professor of Polymer Chemistry at Kyoto University in Japan, as a scientific means to measure, in an objective and reproducible way, the "hand" of textile fabrics. This is achieved by measuring basic mechanical properties that have been correlated with aesthetic properties related to hand (e.g. smoothness, fullness, stiffness, softness, flexibility, and crispness), using a set of four highly specialized measuring devices that were developed specifically for use with the Kawabata System. Those devices are as follows:

Kawabata Tensile and Shear Tester (KES FB1)

Kawabata Pure Bending Tester (KES FB2)

Kawabata Compression Tester (KES FB3)

Kawabata Surface Tester (KES FB4)

KES FB1 through 3 are manufactured by the Kato Iron Works Col., Ltd., Div. Of Instrumentation, Kyoto, Japan. KES FB4 (Kawabata Surface Tester) is manufactured by the Kato Tekko Co., Ltd., Div. Of Instrumentation, Kyoto, Japan. In each case, the measurements were performed according to the standard Kawabata Test Procedures, with 4 8-inchx8-inch samples of each type of fabric being tested, and the results averaged. Care was taken to avoid folding, wrinkling, stressing, or otherwise handling the samples in a way that would deform the sample. The fabric were tested in their as-manufactured form (i.e. they had not undergone subsequent launderings). The die used to cut each sample was aligned with the yarns in the fabric to improve the accuracy of the measurements.

15

### Tensile and Shear Measurements

The testing equipment was set up according to the instructions in the Kawabata manual. The Kawabata shear tester (KES FB1) was allowed to warm up for at least 15 minutes before being calibrated. The tester was set up as follows:

Sensitivity: 2 and  $\times 5$

Sample width: 20 cm

Shear weight: 195 g

Tensile Rate: 0.2 mm/s

Elongation Sensitivity: 25 mm

The shear test measures the resistive forces when the fabric is given a constant tensile force and is subjected to a shear deformation in the direction perpendicular to the constant tensile force.

Mean Shear Stiffness (G) [gf/(cm-deg)]. A lower value for shear stiffness is indicative of more supple hand.

Shear Hysteresis at 0.5°, 2.5° and 50°—(2HG05, 2HG25, and 2HG50, respectively) [gf/cm]—A lower value indicates that the fabric recovers more completely from shear deformation. This correlates to a more supple hand.

Residual Shear Angle at 0.5°, 2.5°, and 5.0° (RG05, RG25, and RG50, respectively). [degrees] The lower the number, the more "return energy" required to return the fabric to its original orientation.

Tensile Energy (WT)—Tensile work (energy) during extension [gf/cm].

Linearity of Extension (LT)—Compares extension work with the work along a hypothetical straight line from (O, y(O)) to (X<sub>Max</sub>, Y(X<sub>Max</sub>)).

Tensile Resilience (RT) [%] Ability to recover from tensile deformation. Lower values mean fabric deformation is more permanent.

% Extensibility (EMT)—% strain (extension) at 500 gf/cm  
[%] Higher number equals more stretch.

### Surface Test

The testing equipment was set up according to the instructions in the Kawabata Manual. The Kawabata Surface Tester (KES FB4) was allowed to warm up for at least 15 minutes before being calibrated. The tester was set up as follows:

Sensitivity 1: 2 and  $\times 5$

Sensitivity 2: 2 and  $\times 5$

Tension Weight: 480 g

Surface Roughness Weight: 10 g

Sample Size: 20x20 cm

The surface test measures frictional properties and geometric roughness properties of the surface of the fabric.

Coefficient of Friction (MIU)—Mean coefficient of friction [dimensionless]. A lower coefficient of friction indicates lower resistance and a smoother hand.

## 15

Surface Roughness (SMD)—Mean deviation of the displacement of contactor normal to surface [microns]. Indicative of the roughness of the fabric surface. High SMD values are associated with poor hand.

Mean Deviation of Coefficient of Friction (MMD) [dimensionless].

## Bending

The testing equipment was set up according to the instructions in the Kawabata Manual. The Kawabata Bending Tester (KES FB2) was allowed to warm up for at least 15 minutes before being calibrated. The tester was set up as follows:

Sensitivity: 2 and  $\times 1$

Sample Size: 20 $\times$ 20 cm

The bending test measures the resistive force encountered when a piece of fabric that is held or anchored in a line parallel to the warp or filling is bent in an arc. The fabric is bent first in the direction of one side and then in the direction of the other side. This action produces a hysteresis curve since the resistive force is measured during bending and unbending in the direction of each side. The width of the fabric in the direction parallel to the bending axis affects the force. The test ultimately measures the bending momentum and bending curvature.

Bending Stiffness (B)—Mean bending stiffness per unit width [gf-cm<sup>2</sup>/cm]. A higher mean bending stiffness indicates a more rigid fabric.

Mean width of bending hysteresis per unit width at K=0.05 cm<sup>-1</sup>, 0.10 cm<sup>-1</sup>, and 0.15 cm<sup>-1</sup> (2HB05, 2HB10, 2HB15, respectively) [gf-cm<sup>2</sup>/cm]. Lower value means the fabric recovers more completely from bending.

Residual bending curvature at K=0.05 cm<sup>-1</sup> (RB05) [cm<sup>-1</sup>]. A lower number indicates a more rigid fabric. RB05 is inversely related to B.

Four samples were tested in each of the warp and filling directions, averaged, and the results are listed in the attached results tables.

## Compression

The testing equipment was set up according to the instructions in the Kawabata manual. The Kawabata Compression Tester (KES FB3) was allowed to warm up for at least 15 minutes before being calibrated. The tester was set up as follows:

Sensitivity: 2 and  $\times 5$

Stroke: 5 mm

Compression Rate: 1 mm/50 s

Sample Size: 20 $\times$ 20 cm

The compression test measured the resistive forces experienced by a plunger having a certain surface area as it moves alternately toward and away from a fabric sample in a direction perpendicular to the fabric. The test ultimately measures the work done in compressing the fabric (forward direction) to a preset maximum force and the work done while decompressing the fabric (reverse direction).

% Compressibility—0.5 grams (COMP) A larger value indicates the fabric has more loft.

Minimum Density—0.5 grams (DMIN) Fabric density at thickness TMIN[g/cm<sup>3</sup>] A less dense fabric is usually more supple and soft.

Maximum Density—50 grams (DMAX) Fabric density at thickness TMAX[g/cm<sup>3</sup>] A less dense fabric is usually more supple and soft.

## 16

Linearity of Compression—(LC) Compares compression work with the work along a hypothetical straight line from (X<sub>0</sub>, y(X<sub>0</sub>)) to (X<sub>max</sub>, y(X<sub>max</sub>)). The larger the value, the more linear the compression. This indicates that the fabric is more isotropic in behavior.

Compressional Resilience (RC) [%] A higher number indicates a more spongy fabric (i.e. it pushes back, indicating loft).

Minimum Thickness—0.5 grams (TMIN)—Thickness [mm] at minimum gf/cm<sup>2</sup>.

Maximum Thickness (TMAX)—Thickness [mm] at maximum pressure (nominal is 50 gf/cm<sup>2</sup>).

Total Thickness Change during Compression (TDIFF) [mm]—Difference of TMIN-TMAX. Indicates the total thickness change during compression.

Compressional Energy (WC)—Energy to compress fabric to 50 gf/cm<sup>2</sup>[gf-cm/cm<sup>2</sup>]. A higher number means that the fabric has more loft and is able to retain more loft during compression.

Decompressional Energy (WC')—This is an indication of the resilience of the fabric, with a larger number indicating greater resiliency.

Weight—[mg/cm<sup>3</sup>]

Although specific examples have been described herein, it is noted that different fabric construction methods (including but not limited to woven, knit, nonwoven, and combinations thereof), can be used within the scope of the invention, as can different types of yarns and combinations thereof including spun yarns (including but not limited to open end spun, air jet spun, ring spun, vortex spun, core spun, compact ring spun, friction spun, and siro spun), filament yarns, and combinations thereof. Likewise, varying fabric weights can be used, as can dyed and undyed fabrics. The fabrics can be used in any number of end products, including but not limited to apparel, industrial, automotive, home furnishings and interiors, composites, etc.

Fabrics according to the invention can be dyed or undyed. One example of a process for producing a dyed fabric is as follows: The fabric can be face finished in the manner described in Ex. 6C while in its greige state, prepared by desizing and scouring in a conventional manner, heatsetting under normal processing conditions for these types of fabrics (as will be readily appreciated by those of ordinary skill in the art), dyed in a thermosol at 425 degrees Fahrenheit, and a conventional chemical finish designed to enhance the fabric's soil release characteristics can be applied.

TABLE B

|                                | Tensile Analysis Summary |        |        |        |        |        |       |          |
|--------------------------------|--------------------------|--------|--------|--------|--------|--------|-------|----------|
|                                | A                        | B      | C      | D      | Avg    | STD    | ERR   |          |
| Example 9A - Warp Direction    |                          |        |        |        |        |        |       |          |
| 55                             | WT                       | 4.254  | 5.910  | 3.996  | 4.018  | 4.545  | 0.918 | +/-1.459 |
|                                | LT                       | 0.677  | 0.733  | 0.764  | 0.654  | 0.707  | 0.050 | +/-0.080 |
|                                | RT                       | 57.766 | 49.906 | 58.383 | 59.881 | 56.484 | 4.474 | +/-7.114 |
|                                | EMT                      | 2.475  | 3.195  | 2.060  | 2.420  | 2.538  | 0.475 | +/-0.756 |
| Example 9A - Filling Direction |                          |        |        |        |        |        |       |          |
| 55                             | WT                       | 12.383 | 10.753 | 10.101 | 9.270  | 10.627 | 1.319 | +/-2.097 |
|                                | LT                       | 0.618  | 0.569  | 0.660  | 0.659  | 0.627  | 0.043 | +/-0.068 |
|                                | RT                       | 50.194 | 57.866 | 55.236 | 56.005 | 54.825 | 3.279 | +/-5.214 |
|                                | EMT                      | 7.900  | 7.450  | 6.030  | 5.595  | 6.744  | 1.105 | +/-1.757 |
| Example 9B - Warp Direction    |                          |        |        |        |        |        |       |          |
| 65                             | WT                       | 4.448  | 4.032  | 4.615  | 3.648  | 4.186  | 0.434 | +/-0.691 |
|                                | LT                       | 0.595  | 0.685  | 0.818  | 0.629  | 0.682  | 0.098 | +/-0.156 |
|                                | RT                       | 58.430 | 57.344 | 56.102 | 66.670 | 59.637 | 4.784 | +/-7.607 |

TABLE B-continued

| Tensile Analysis Summary       |        |        |        |        |        |       |          |
|--------------------------------|--------|--------|--------|--------|--------|-------|----------|
|                                | A      | B      | C      | D      | Avg    | STD   | ERR      |
| EMT                            | 2.915  | 2.330  | 2.235  | 2.275  | 2.439  | 0.320 | +/-0.509 |
| Example 9B - Filling Direction |        |        |        |        |        |       |          |
| WT                             | 10.604 | 10.384 | 10.957 | 10.130 | 10.519 | 0.351 | +/-0.557 |
| LT                             | 0.591  | 0.651  | 0.658  | 0.616  | 0.629  | 0.031 | +/-0.050 |
| RT                             | 57.001 | 55.111 | 52.542 | 56.030 | 55.171 | 1.915 | +/-3.045 |
| EMT                            | 7.070  | 6.285  | 6.535  | 6.515  | 6.601  | 0.332 | +/-0.529 |
| Example 9C - Warp Direction    |        |        |        |        |        |       |          |
| WT                             | 3.694  | 3.014  | 3.315  | 3.392  | 3.354  | 0.279 | +/-0.444 |
| LT                             | 0.658  | 0.779  | 0.693  | 0.679  | 0.702  | 0.053 | +/-0.085 |

TABLE B-continued

| Tensile Analysis Summary       |        |        |        |        |        |       |          |
|--------------------------------|--------|--------|--------|--------|--------|-------|----------|
|                                | A      | B      | C      | D      | Avg    | STD   | ERR      |
| RT                             | 57.385 | 56.647 | 59.678 | 60.260 | 58.493 | 1.748 | +/-2.779 |
| EMT                            | 2.170  | 1.525  | 1.875  | 1.950  | 1.880  | 0.268 | +/-0.426 |
| Example 9C - Filling Direction |        |        |        |        |        |       |          |
| WT                             | 8.061  | 8.438  | 8.178  | 12.583 | 9.315  | 2.184 | +/-3.473 |
| LT                             | 0.700  | 0.679  | 0.611  | 0.928  | 0.730  | 0.138 | +/-0.219 |
| RT                             | 54.754 | 50.960 | 52.963 | 49.927 | 52.151 | 2.145 | +/-3.410 |
| EMT                            | 4.495  | 4.870  | 5.250  | 4.930  | 4.886  | 0.310 | +/-0.492 |

TABLE C

| COMPRESSION ANALYSIS SUMMARY |        |        |        |        |        |       |          |
|------------------------------|--------|--------|--------|--------|--------|-------|----------|
|                              | A      | B      | C      | D      | Avg    | STD   | ERR      |
| Example 9A                   |        |        |        |        |        |       |          |
| Comp                         | 35.170 | 39.676 | 33.898 | 36.082 | 36.207 | 2.480 | +/-3.944 |
| Densitymin                   | 0.272  | 0.251  | 0.278  | 0.276  | 0.269  | 0.012 | +/-0.020 |
| Densitymax                   | 0.420  | 0.417  | 0.420  | 0.432  | 0.422  | 0.007 | +/-0.011 |
| LC                           | 0.340  | 0.314  | 0.346  | 0.332  | 0.333  | 0.014 | +/-0.022 |
| RC                           | 54.029 | 52.059 | 51.791 | 52.325 | 52.551 | 1.009 | +/-1.605 |
| Tmin                         | 0.545  | 0.586  | 0.531  | 0.534  | 0.549  | 0.025 | +/-0.040 |
| Tdiff                        | 0.192  | 0.233  | 0.180  | 0.193  | 0.200  | 0.023 | +/-0.037 |
| Tmax                         | 0.353  | 0.354  | 0.351  | 0.341  | 0.350  | 0.006 | +/-0.009 |
| WC                           | 0.165  | 0.180  | 0.153  | 0.161  | 0.165  | 0.011 | +/-0.018 |
| WCPrime                      | 0.089  | 0.094  | 0.079  | 0.084  | 0.087  | 0.006 | +/-0.010 |
| Weight                       | 14.825 | 14.725 | 14.750 | 14.725 | 14.756 | 0.047 | +/-0.075 |
| Example 9B                   |        |        |        |        |        |       |          |
| Comp                         | 37.804 | 35.433 | 34.232 | 39.337 | 36.702 | 2.300 | +/-3.657 |
| Densitymin                   | 0.266  | 0.290  | 0.295  | 0.265  | 0.279  | 0.016 | +/-0.025 |
| Densitymax                   | 0.428  | 0.449  | 0.449  | 0.436  | 0.441  | 0.010 | +/-0.016 |
| LC                           | 0.354  | 0.313  | 0.326  | 0.325  | 0.330  | 0.017 | +/-0.028 |
| RC                           | 49.227 | 53.947 | 52.646 | 51.271 | 51.773 | 2.018 | +/-3.209 |
| Tmin                         | 0.556  | 0.508  | 0.501  | 0.558  | 0.531  | 0.030 | +/-0.048 |
| Tdiff                        | 0.210  | 0.180  | 0.171  | 0.219  | 0.195  | 0.023 | +/-0.037 |
| Tmax                         | 0.346  | 0.328  | 0.330  | 0.339  | 0.336  | 0.008 | +/-0.013 |
| WC                           | 0.185  | 0.137  | 0.142  | 0.181  | 0.161  | 0.025 | +/-0.040 |
| WCPrime                      | 0.091  | 0.074  | 0.075  | 0.093  | 0.083  | 0.010 | +/-0.016 |
| Weight                       | 14.775 | 14.725 | 14.800 | 14.775 | 14.769 | 0.031 | +/-0.050 |
| Example 9C                   |        |        |        |        |        |       |          |
| Comp                         | 55.972 | 53.197 | 57.062 | 52.468 | 54.675 | 2.194 | +/-3.488 |
| Densitymin                   | 0.225  | 0.235  | 0.211  | 0.237  | 0.227  | 0.012 | +/-0.019 |
| Densitymax                   | 0.512  | 0.502  | 0.491  | 0.498  | 0.501  | 0.009 | +/-0.014 |
| LC                           | 0.276  | 0.296  | 0.277  | 0.293  | 0.286  | 0.010 | +/-0.017 |
| RC                           | 47.473 | 49.672 | 47.469 | 48.692 | 48.327 | 1.066 | +/-1.695 |
| Tmin                         | 0.653  | 0.634  | 0.705  | 0.628  | 0.655  | 0.035 | +/-0.056 |
| Tdiff                        | 0.366  | 0.337  | 0.402  | 0.330  | 0.359  | 0.033 | +/-0.052 |
| Tmax                         | 0.288  | 0.297  | 0.303  | 0.299  | 0.297  | 0.006 | +/-0.010 |
| WC                           | 0.248  | 0.248  | 0.277  | 0.240  | 0.253  | 0.016 | +/-0.026 |
| WCPrime                      | 0.118  | 0.123  | 0.132  | 0.117  | 0.123  | 0.007 | +/-0.011 |
| Weight                       | 14.725 | 14.875 | 14.850 | 14.875 | 14.831 | 0.072 | +/-0.114 |

TABLE D

| SHEAR ANALYSIS SUMMARY      |       |       |       |       |       |       |          |
|-----------------------------|-------|-------|-------|-------|-------|-------|----------|
|                             | A     | B     | C     | D     | Avg   | STD   | ERR      |
| Example 9A - Warp Direction |       |       |       |       |       |       |          |
| G                           | 0.832 | 0.889 | 1.001 | 0.952 | 0.919 | 0.074 | +/-0.117 |
| 2HG05                       | 1.512 | 1.625 | 1.757 | 1.533 | 1.607 | 0.112 | +/-0.177 |
| 2HG25                       | 2.244 | 2.461 | 2.728 | 2.582 | 2.504 | 0.205 | +/-0.325 |
| 2HG50                       | 3.503 | 3.702 | 4.178 | 4.246 | 3.907 | 0.362 | +/-0.576 |

TABLE D-continued

| SHEAR ANALYSIS SUMMARY                |        |        |        |        |        |       |          |
|---------------------------------------|--------|--------|--------|--------|--------|-------|----------|
|                                       | A      | B      | C      | D      | Avg    | STD   | ERR      |
| RG05                                  | 1.819  | 1.828  | 1.755  | 1.611  | 1.753  | 0.100 | +/-0.159 |
| RG25                                  | 2.699  | 2.769  | 2.725  | 2.714  | 2.727  | 0.030 | +/-0.048 |
| RG50                                  | 4.212  | 4.165  | 4.172  | 4.463  | 4.253  | 0.142 | +/-0.225 |
| <u>Example 9A - Filling Direction</u> |        |        |        |        |        |       |          |
| G                                     | 0.444  | 0.739  | 0.866  | 0.757  | 0.702  | 0.181 | +/-0.287 |
| 2HG05                                 | 0.958  | 1.192  | 1.183  | 1.227  | 1.140  | 0.123 | +/-0.195 |
| 2HG25                                 | 1.509  | 1.913  | 2.126  | 1.913  | 1.865  | 0.258 | +/-0.410 |
| 2HG50                                 | 2.987  | 3.270  | 3.818  | 3.576  | 3.413  | 0.362 | +/-0.575 |
| RG05                                  | 2.156  | 1.612  | 1.365  | 1.621  | 1.689  | 0.333 | +/-0.530 |
| RG25                                  | 3.396  | 2.588  | 2.455  | 2.527  | 2.742  | 0.440 | +/-0.699 |
| RG50                                  | 6.722  | 4.423  | 4.408  | 4.723  | 5.069  | 1.112 | +/-1.767 |
| <u>Example 9B - Warp Direction</u>    |        |        |        |        |        |       |          |
| G                                     | 1.091  | 1.412  | 1.330  | 1.099  | 1.233  | 0.163 | +/-0.259 |
| 2HG05                                 | 1.401  | 1.835  | 1.656  | 1.561  | 1.613  | 0.181 | +/-0.289 |
| 2HG25                                 | 2.563  | 3.325  | 3.162  | 2.629  | 2.920  | 0.381 | +/-0.605 |
| 2HG50                                 | 4.238  | 5.322  | 5.258  | 4.419  | 4.809  | 0.561 | +/-0.891 |
| RG05                                  | 1.284  | 1.299  | 1.245  | 1.420  | 1.312  | 0.076 | +/-0.120 |
| RG25                                  | 2.350  | 2.354  | 2.378  | 2.392  | 2.369  | 0.020 | +/-0.032 |
| RG50                                  | 3.886  | 3.769  | 3.953  | 4.021  | 3.907  | 0.107 | +/-0.171 |
| <u>Example 9C - Warp Direction</u>    |        |        |        |        |        |       |          |
| G                                     | 0.861  | 1.193  | 1.086  | 0.946  | 1.022  | 0.147 | +/-0.234 |
| 2HG05                                 | 1.209  | 1.135  | 1.372  | 1.283  | 1.250  | 0.101 | +/-0.161 |
| 2HG25                                 | 2.042  | 2.611  | 2.486  | 2.292  | 2.358  | 0.248 | +/-0.394 |
| 2HG50                                 | 3.713  | 4.924  | 4.528  | 4.065  | 4.308  | 0.529 | +/-0.842 |
| RG05                                  | 1.405  | 0.951  | 1.264  | 1.356  | 1.244  | 0.204 | +/-0.324 |
| RG25                                  | 2.373  | 2.188  | 2.290  | 2.422  | 2.318  | 0.103 | +/-0.163 |
| RG50                                  | 4.315  | 4.127  | 4.171  | 4.295  | 4.227  | 0.092 | +/-0.147 |
| <u>Example 9C - Filling Direction</u> |        |        |        |        |        |       |          |
| G                                     | 3.112  | 3.135  | 3.592  | 3.126  | 3.241  | 0.234 | +/-0.372 |
| 2HG05                                 | 1.636  | 1.774  | 2.563  | 1.908  | 1.970  | 0.410 | +/-0.653 |
| 2HG25                                 | 6.332  | 6.665  | 7.666  | 6.704  | 6.842  | 0.574 | +/-0.913 |
| 2HG50                                 | 10.966 | 12.022 | 11.951 | 12.262 | 11.800 | 0.572 | +/-0.909 |
| RG05                                  | 0.526  | 0.566  | 0.714  | 0.610  | 0.604  | 0.081 | +/-0.129 |
| RG25                                  | 2.035  | 2.126  | 2.134  | 2.144  | 2.110  | 0.050 | +/-0.080 |
| RG50                                  | 3.524  | 3.835  | 3.327  | 3.922  | 3.652  | 0.276 | +/-0.439 |
| <u>Example 9C - Filling Direction</u> |        |        |        |        |        |       |          |
| G                                     | 3.494  | 2.885  | 3.792  | 3.268  | 3.360  | 0.382 | +/-0.608 |
| 2HG05                                 | 1.849  | 1.896  | 2.123  | 1.655  | 1.881  | 0.192 | +/-0.306 |
| 2HG25                                 | 7.250  | 6.231  | 7.994  | 6.837  | 7.078  | 0.740 | +/-1.177 |
| 2HG50                                 | 14.060 | 11.321 | 14.225 | 13.735 | 13.335 | 1.358 | +/-2.159 |
| RG05                                  | 0.529  | 0.657  | 0.560  | 0.506  | 0.563  | 0.066 | +/-0.106 |
| RG25                                  | 2.075  | 2.159  | 2.108  | 2.092  | 2.109  | 0.036 | +/-0.058 |
| RG50                                  | 4.024  | 3.924  | 3.751  | 4.202  | 3.975  | 0.189 | +/-0.300 |

TABLE E

| Surface Analysis Summary              |       |       |       |       |       |       | 50       | Surface Analysis Summary              |     |       |       |       |       |       |       |          |
|---------------------------------------|-------|-------|-------|-------|-------|-------|----------|---------------------------------------|-----|-------|-------|-------|-------|-------|-------|----------|
|                                       | A     | B     | C     | D     | Avg   | STD   | ERR      |                                       | A   | B     | C     | D     | Avg   | STD   | ERR   |          |
| <u>Example 9A - Warp Direction</u>    |       |       |       |       |       |       |          | <u>Example 9B - Filling Direction</u> |     |       |       |       |       |       |       |          |
| MIU                                   | 0.236 | 0.223 | 0.224 | 0.222 | 0.226 | 0.007 | +/-0.010 | 55                                    | MIU | 0.226 | 0.222 | 0.224 | 0.226 | 0.225 | 0.002 | +/-0.003 |
| MMD                                   | 0.069 | 0.076 | 0.085 | 0.084 | 0.079 | 0.008 | +/-0.012 |                                       | MMD | 0.041 | 0.044 | 0.046 | 0.042 | 0.043 | 0.002 | +/-0.004 |
| SMD                                   | 8.190 | 6.473 | 6.327 | 6.573 | 6.891 | 0.872 | +/-1.387 |                                       | SMD | 4.614 | 4.378 | 5.429 | 4.242 | 4.666 | 0.532 | +/-0.845 |
| <u>Example 9A - Filling Direction</u> |       |       |       |       |       |       |          | <u>Example 9C - Warp Direction</u>    |     |       |       |       |       |       |       |          |
| MIU                                   | 0.229 | 0.229 | 0.223 | 0.230 | 0.228 | 0.003 | +/-0.005 | 60                                    | MIU | 0.197 | 0.195 | 0.202 | 0.208 | 0.201 | 0.006 | +/-0.009 |
| MMD                                   | 0.032 | 0.036 | 0.040 | 0.024 | 0.033 | 0.007 | +/-0.011 |                                       | MMD | 0.052 | 0.055 | 0.049 | 0.044 | 0.050 | 0.005 | +/-0.007 |
| SMD                                   | 3.049 | 3.651 | 4.506 | 4.719 | 3.981 | 0.774 | +/-1.231 |                                       | SMD | 6.558 | 6.161 | 7.167 | 7.180 | 6.767 | 0.497 | +/-0.790 |
| <u>Example 9B - Warp Direction</u>    |       |       |       |       |       |       |          | <u>Example 9C - Filling Direction</u> |     |       |       |       |       |       |       |          |
| MIU                                   | 0.227 | 0.221 | 0.219 | 0.217 | 0.221 | 0.004 | +/-0.007 |                                       | MIU | 0.199 | 0.207 | 0.215 | 0.219 | 0.210 | 0.009 | +/-0.014 |
| MMD                                   | 0.076 | 0.080 | 0.067 | 0.072 | 0.074 | 0.006 | +/-0.009 | 65                                    | MMD | 0.060 | 0.048 | 0.057 | 0.051 | 0.054 | 0.005 | +/-0.009 |
| SMD                                   | 7.201 | 6.495 | 7.950 | 8.453 | 7.525 | 0.858 | +/-1.364 |                                       | SMD | 5.544 | 4.609 | 4.354 | 4.433 | 4.735 | 0.550 | +/-0.874 |

TABLE F

| Bending Analysis Summary              |       |       |       |       |       |       |          |
|---------------------------------------|-------|-------|-------|-------|-------|-------|----------|
|                                       | A     | B     | C     | D     | Avg   | STD   | ERR      |
| <u>Example 9A - Warp Direction</u>    |       |       |       |       |       |       |          |
| B                                     | 0.066 | 0.080 | 0.078 | 0.086 | 0.078 | 0.008 | +/-0.013 |
| 2HB05                                 | 0.070 | 0.071 | 0.085 | 0.077 | 0.076 | 0.007 | +/-0.011 |
| 2HB10                                 | 0.077 | 0.085 | 0.096 | 0.094 | 0.088 | 0.009 | +/-0.014 |
| 2HB15                                 | 0.080 | 0.093 | 0.101 | 0.103 | 0.094 | 0.010 | +/-0.017 |
| RB05                                  | 1.060 | 0.892 | 1.086 | 0.896 | 0.984 | 0.104 | +/-0.165 |
| RB10                                  | 1.167 | 1.062 | 1.237 | 1.092 | 1.140 | 0.079 | +/-0.125 |
| RB15                                  | 1.213 | 1.163 | 1.293 | 1.196 | 1.216 | 0.055 | +/-0.088 |
| <u>Example 9A - Filling Direction</u> |       |       |       |       |       |       |          |
| B                                     | 0.052 | 0.083 | 0.111 | 0.087 | 0.083 | 0.024 | +/-0.039 |
| 2HB05                                 | 0.045 | 0.066 | 0.073 | 0.089 | 0.068 | 0.018 | +/-0.029 |
| 2HB10                                 | 0.051 | 0.083 | 0.097 | 0.100 | 0.083 | 0.022 | +/-0.036 |
| 2HB15                                 | 0.059 | 0.094 | 0.113 | 0.109 | 0.094 | 0.025 | +/-0.039 |
| RB05                                  | 0.880 | 0.792 | 0.660 | 1.029 | 0.840 | 0.155 | +/-0.246 |
| RB10                                  | 0.998 | 0.993 | 0.875 | 1.160 | 1.007 | 0.117 | +/-0.186 |
| RB15                                  | 1.152 | 1.123 | 1.019 | 1.255 | 1.137 | 0.097 | +/-0.154 |
| <u>Example 9B - Warp Direction</u>    |       |       |       |       |       |       |          |
| B                                     | 0.087 | 0.114 | 0.104 | 0.077 | 0.096 | 0.017 | +/-0.026 |
| 2HB05                                 | 0.090 | 0.081 | 0.104 | 0.079 | 0.089 | 0.011 | +/-0.018 |
| 2HB10                                 | 0.104 | 0.106 | 0.122 | 0.090 | 0.106 | 0.013 | +/-0.021 |
| 2HB15                                 | 0.110 | 0.123 | 0.131 | 0.098 | 0.116 | 0.015 | +/-0.023 |
| RB05                                  | 1.033 | 0.713 | 0.999 | 1.023 | 0.942 | 0.153 | +/-0.244 |
| RB10                                  | 1.191 | 0.935 | 1.176 | 1.174 | 1.119 | 0.123 | +/-0.195 |
| RB15                                  | 1.257 | 1.087 | 1.262 | 1.268 | 1.219 | 0.088 | +/-0.140 |
| <u>Example 9B - Filling Direction</u> |       |       |       |       |       |       |          |
| B                                     | 0.081 | 0.109 | 0.084 | 0.073 | 0.087 | 0.016 | +/-0.025 |
| 2HB05                                 | 0.071 | 0.097 | 0.082 | 0.068 | 0.080 | 0.013 | +/-0.021 |
| 2HB10                                 | 0.091 | 0.120 | 0.101 | 0.085 | 0.099 | 0.015 | +/-0.024 |
| 2HB15                                 | 0.103 | 0.136 | 0.110 | 0.095 | 0.111 | 0.018 | +/-0.028 |
| RB05                                  | 0.872 | 0.888 | 0.976 | 0.935 | 0.918 | 0.047 | +/-0.075 |
| RB10                                  | 1.121 | 1.104 | 1.197 | 1.171 | 1.148 | 0.043 | +/-0.069 |
| RB15                                  | 1.272 | 1.246 | 1.305 | 1.299 | 1.281 | 0.027 | +/-0.043 |
| <u>Example 9C - Warp Direction</u>    |       |       |       |       |       |       |          |
| B                                     | 0.123 | 0.114 | 0.258 | 0.150 | 0.161 | 0.066 | +/-0.105 |
| 2HB05                                 | 0.083 | 0.082 | 0.166 | 0.099 | 0.108 | 0.040 | +/-0.063 |
| 2HB10                                 | 0.109 | 0.102 | 0.224 | 0.126 | 0.140 | 0.057 | +/-0.090 |
| 2HB15                                 | 0.135 | 0.124 | 0.285 | 0.156 | 0.175 | 0.075 | +/-0.118 |
| RB05                                  | 0.676 | 0.719 | 0.644 | 0.660 | 0.675 | 0.032 | +/-0.051 |
| RB10                                  | 0.882 | 0.900 | 0.870 | 0.842 | 0.874 | 0.024 | +/-0.039 |
| RB15                                  | 1.092 | 1.092 | 1.105 | 1.041 | 1.083 | 0.028 | +/-0.045 |
| <u>Example 9C - Filling Direction</u> |       |       |       |       |       |       |          |
| B                                     | 0.201 | 0.110 | 0.118 | 0.109 | 0.135 | 0.045 | +/-0.071 |
| 2HB05                                 | 0.146 | 0.086 | 0.104 | 0.099 | 0.109 | 0.026 | +/-0.041 |
| 2HB10                                 | 0.191 | 0.108 | 0.127 | 0.118 | 0.136 | 0.037 | +/-0.060 |
| 2HB15                                 | 0.239 | 0.130 | 0.148 | 0.140 | 0.164 | 0.050 | +/-0.080 |
| RB05                                  | 0.726 | 0.780 | 0.876 | 0.908 | 0.823 | 0.084 | +/-0.134 |
| RB10                                  | 0.954 | 0.975 | 1.072 | 1.090 | 1.023 | 0.068 | +/-0.108 |
| RB15                                  | 1.190 | 1.175 | 1.252 | 1.287 | 1.226 | 0.053 | +/-0.084 |

TABLE G

| Tensile Analysis Summary               |       |        |        |        |        |        |          |
|----------------------------------------|-------|--------|--------|--------|--------|--------|----------|
|                                        | A     | B      | C      | D      | Avg    | STD    | ERR      |
| <u>Example 10A - Warp Direction</u>    |       |        |        |        |        |        |          |
| 5                                      | WT    | 4.597  | 4.621  | 4.671  | 4.943  | 4.708  | 0.160    |
| 10                                     | WT    | 10.810 | 10.407 | 9.780  | 10.567 | 10.391 | 0.440    |
| 15                                     | WT    | 4.242  | 4.522  | 4.677  | 4.383  | 4.456  | 0.186    |
| 20                                     | WT    | 0.364  | 0.686  | 0.720  | 0.736  | 0.627  | 0.176    |
| 25                                     | WT    | 4.620  | 2.585  | 2.535  | 2.335  | 3.019  | 1.073    |
| 30                                     | WT    | 10.528 | 9.927  | 9.688  | 9.800  | 9.986  | 0.374    |
| 35                                     | WT    | 0.650  | 0.581  | 0.637  | 0.611  | 0.620  | 0.030    |
| 40                                     | WT    | 59.322 | 62.614 | 57.958 | 61.279 | 60.293 | 2.062    |
| 45                                     | WT    | 4.213  | 4.412  | 4.351  | 4.532  | 4.377  | 0.133    |
| 50                                     | WT    | 0.679  | 0.607  | 0.849  | 0.663  | 0.700  | 0.104    |
| <u>Example 10B - Warp Direction</u>    |       |        |        |        |        |        |          |
| EMT                                    | 6.955 | 6.515  | 5.875  | 7.890  | 6.809  | 0.846  | +/-0.346 |
| <u>Example 10B - Filling Direction</u> |       |        |        |        |        |        |          |
| EMT                                    | 6.350 | 6.700  | 5.960  | 6.290  | 6.325  | 0.303  | +/-0.482 |
| <u>Example 10C - Warp Direction</u>    |       |        |        |        |        |        |          |
| EMT                                    | 1.470 | 1.110  | 1.445  | 1.445  | 1.368  | 0.172  | +/-0.274 |
| <u>Example 10C - Filling Direction</u> |       |        |        |        |        |        |          |
| EMT                                    | 2.445 | 2.850  | 1.980  | 2.680  | 2.489  | 0.378  | +/-0.600 |

TABLE H

| COMPRESSION ANALYSIS SUMMARY |        |        |        |        |        |       |          |
|------------------------------|--------|--------|--------|--------|--------|-------|----------|
|                              | A      | B      | C      | D      | Avg    | STD   | ERR      |
| <u>Example 10A</u>           |        |        |        |        |        |       |          |
| Comp                         | 26.502 | 25.186 | 30.826 | 32.763 | 28.819 | 3.566 | +/-5.670 |
| Densitymin                   | 0.329  | 0.342  | 0.308  | 0.290  | 0.317  | 0.023 | +/-0.036 |
| Densitymax                   | 0.447  | 0.457  | 0.446  | 0.431  | 0.445  | 0.011 | +/-0.017 |
| LC                           | 0.337  | 0.354  | 0.310  | 0.327  | 0.332  | 0.018 | +/-0.029 |

TABLE H-continued

| COMPRESSION ANALYSIS SUMMARY |        |        |        |        |        |       |          |
|------------------------------|--------|--------|--------|--------|--------|-------|----------|
|                              | A      | B      | C      | D      | Avg    | STD   | ERR      |
| RC                           | 47.255 | 46.782 | 45.160 | 43.529 | 45.682 | 1.692 | +/-2.691 |
| Tmin                         | 0.708  | 0.673  | 0.745  | 0.789  | 0.729  | 0.050 | +/-0.079 |
| Tdiff                        | 0.187  | 0.169  | 0.229  | 0.258  | 0.211  | 0.040 | +/-0.064 |
| Tmax                         | 0.520  | 0.504  | 0.515  | 0.531  | 0.518  | 0.011 | +/-0.018 |
| WC                           | 0.158  | 0.148  | 0.175  | 0.213  | 0.174  | 0.029 | +/-0.045 |
| WCPrime                      | 0.075  | 0.069  | 0.079  | 0.093  | 0.079  | 0.010 | +/-0.016 |
| Weight                       | 23.250 | 23.000 | 22.950 | 22.875 | 23.019 | 0.162 | +/-0.258 |
| Example 10B                  |        |        |        |        |        |       |          |
| Comp                         | 34.201 | 33.661 | 33.553 | 33.157 | 33.643 | 0.430 | +/-0.684 |
| Densitymin                   | 0.296  | 0.299  | 0.300  | 0.301  | 0.299  | 0.002 | +/-0.003 |
| Densitymax                   | 0.450  | 0.450  | 0.452  | 0.450  | 0.451  | 0.001 | +/-0.002 |
| LC                           | 0.321  | 0.327  | 0.338  | 0.343  | 0.332  | 0.010 | +/-0.016 |
| RC                           | 47.961 | 48.526 | 48.817 | 48.715 | 48.505 | 0.382 | +/-0.607 |
| Tmin                         | 0.788  | 0.762  | 0.760  | 0.756  | 0.767  | 0.015 | +/-0.023 |
| Tdiff                        | 0.269  | 0.256  | 0.255  | 0.250  | 0.258  | 0.008 | +/-0.013 |
| Tmax                         | 0.519  | 0.506  | 0.505  | 0.505  | 0.509  | 0.007 | +/-0.011 |
| WC                           | 0.212  | 0.207  | 0.214  | 0.212  | 0.211  | 0.003 | +/-0.005 |
| WCPrime                      | 0.102  | 0.100  | 0.104  | 0.103  | 0.102  | 0.002 | +/-0.003 |
| Weight                       | 23.350 | 22.750 | 22.825 | 22.750 | 22.919 | 0.290 | +/-0.461 |
| Example 10C                  |        |        |        |        |        |       |          |
| Comp                         | 37.784 | 41.531 | 39.912 | 40.853 | 40.020 | 1.632 | +/-2.595 |
| Densitymin                   | 0.288  | 0.266  | 0.283  | 0.275  | 0.278  | 0.010 | +/-0.015 |
| Densitymax                   | 0.464  | 0.455  | 0.471  | 0.465  | 0.464  | 0.007 | +/-0.010 |
| LC                           | 0.336  | 0.309  | 0.286  | 0.290  | 0.305  | 0.023 | +/-0.036 |
| RC                           | 49.422 | 49.227 | 50.701 | 50.413 | 49.941 | 0.726 | +/-1.154 |
| Tmin                         | 0.772  | 0.830  | 0.796  | 0.809  | 0.802  | 0.024 | +/-0.039 |
| Tdiff                        | 0.291  | 0.344  | 0.318  | 0.331  | 0.321  | 0.023 | +/-0.036 |
| Tmax                         | 0.480  | 0.485  | 0.478  | 0.479  | 0.481  | 0.003 | +/-0.005 |
| WC                           | 0.247  | 0.270  | 0.226  | 0.238  | 0.245  | 0.019 | +/-0.030 |
| WCPrime                      | 0.122  | 0.133  | 0.115  | 0.120  | 0.123  | 0.008 | +/-0.012 |
| Weight                       | 22.250 | 22.050 | 22.500 | 22.250 | 22.263 | 0.184 | +/-0.293 |

TABLE I

| SHEAR ANALYSIS SUMMARY          |       |       |       |       |       |       |          |
|---------------------------------|-------|-------|-------|-------|-------|-------|----------|
|                                 | A     | B     | C     | D     | Avg   | STD   | ERR      |
| Example 10A - Warp Direction    |       |       |       |       |       |       |          |
| G                               | 1.576 | 1.724 | 1.635 | 1.491 | 1.607 | 0.098 | +/-0.156 |
| 2HG05                           | 3.518 | 3.020 | 2.796 | 3.216 | 3.138 | 0.306 | +/-0.487 |
| 2HG25                           | 4.884 | 4.803 | 4.551 | 4.559 | 4.699 | 0.170 | +/-0.270 |
| 2HG50                           | 6.678 | 7.103 | 6.957 | 6.423 | 6.790 | 0.302 | +/-0.480 |
| RG05                            | 2.232 | 1.751 | 1.710 | 2.158 | 1.963 | 0.270 | +/-0.430 |
| RG25                            | 3.100 | 2.785 | 2.783 | 3.058 | 2.932 | 0.171 | +/-0.272 |
| RG50                            | 4.238 | 4.119 | 4.254 | 4.308 | 4.230 | 0.080 | +/-0.127 |
| Example 10A - Filling Direction |       |       |       |       |       |       |          |
| G                               | 1.335 | 1.492 | 1.505 | 1.130 | 1.366 | 0.175 | +/-0.278 |
| 2HG05                           | 2.487 | 2.456 | 2.318 | 2.493 | 2.439 | 0.082 | +/-0.130 |
| 2HG25                           | 3.783 | 4.147 | 4.042 | 3.493 | 3.866 | 0.292 | +/-0.464 |
| 2HG50                           | 6.292 | 7.160 | 7.120 | 5.621 | 6.548 | 0.736 | +/-1.171 |
| RG05                            | 1.863 | 1.645 | 1.541 | 2.206 | 1.814 | 0.294 | +/-0.467 |
| RG25                            | 2.834 | 2.779 | 2.687 | 3.091 | 2.848 | 0.173 | +/-0.275 |
| RG50                            | 4.714 | 4.798 | 4.732 | 4.974 | 4.805 | 0.119 | +/-0.189 |
| Example 10B - Warp Direction    |       |       |       |       |       |       |          |
| G                               | 1.897 | 1.751 | 1.599 | 1.581 | 1.707 | 0.148 | +/-0.235 |
| 2HG05                           | 3.547 | 3.108 | 2.610 | 2.814 | 3.020 | 0.407 | +/-0.647 |
| 2HG25                           | 5.393 | 4.989 | 4.355 | 4.595 | 4.833 | 0.456 | +/-0.725 |
| 2HG50                           | 7.347 | 7.826 | 7.227 | 7.347 | 7.437 | 0.266 | +/-0.422 |
| RG05                            | 1.870 | 1.775 | 1.632 | 1.781 | 1.765 | 0.098 | +/-0.157 |
| RG25                            | 2.843 | 2.849 | 2.724 | 2.907 | 2.831 | 0.077 | +/-0.122 |
| RG50                            | 3.874 | 4.469 | 4.520 | 4.648 | 4.378 | 0.344 | +/-0.547 |
| Example 10B - Filling Direction |       |       |       |       |       |       |          |
| G                               | 1.539 | 1.651 | 1.560 | 1.467 | 1.554 | 0.076 | +/-0.121 |
| 2HG05                           | 2.766 | 2.447 | 2.426 | 2.378 | 2.504 | 0.177 | +/-0.281 |
| 2HG25                           | 4.524 | 4.467 | 4.351 | 4.064 | 4.352 | 0.205 | +/-0.326 |

TABLE I-continued

| SHEAR ANALYSIS SUMMARY          |        |        |        |        |        |       |          |
|---------------------------------|--------|--------|--------|--------|--------|-------|----------|
|                                 | A      | B      | C      | D      | Avg    | STD   | ERR      |
| 2HG50                           | 7.990  | 8.454  | 7.874  | 7.474  | 7.948  | 0.403 | +/-0.641 |
| RG05                            | 1.797  | 1.482  | 1.555  | 1.621  | 1.614  | 0.135 | +/-0.214 |
| RG25                            | 2.940  | 2.705  | 2.790  | 2.770  | 2.801  | 0.099 | +/-0.158 |
| RG50                            | 5.192  | 5.120  | 5.048  | 5.095  | 5.114  | 0.060 | +/-0.096 |
| Example 10C - Warp Direction    |        |        |        |        |        |       |          |
| G                               | 2.834  | 2.335  | 2.655  | 2.469  | 2.573  | 0.218 | +/-0.346 |
| 2HG05                           | 1.797  | 1.677  | 1.412  | 2.059  | 1.736  | 0.269 | +/-0.427 |
| 2HG25                           | 5.998  | 5.136  | 5.408  | 5.601  | 5.536  | 0.362 | +/-0.576 |
| 2HG50                           | 12.732 | 10.724 | 11.645 | 11.247 | 11.587 | 0.851 | +/-1.354 |
| RG05                            | 0.634  | 0.718  | 0.532  | 0.834  | 0.680  | 0.128 | +/-0.204 |
| RG25                            | 2.116  | 2.200  | 2.037  | 2.269  | 2.156  | 0.101 | +/-0.160 |
| RG50                            | 4.492  | 4.593  | 4.386  | 4.555  | 4.507  | 0.090 | +/-0.144 |
| Example 10C - Filling Direction |        |        |        |        |        |       |          |
| G                               | 2.954  | 2.036  | 2.556  | 2.496  | 2.511  | 0.376 | +/-0.598 |
| 2HG05                           | 1.339  | 1.357  | 1.335  | 1.323  | 1.339  | 0.014 | +/-0.022 |
| 2HG25                           | 5.889  | 4.453  | 5.204  | 5.133  | 5.170  | 0.587 | +/-0.933 |
| 2HG50                           | 13.354 | 9.911  | 11.220 | 11.203 | 11.422 | 1.426 | +/-2.268 |
| RG05                            | 0.453  | 0.667  | 0.522  | 0.530  | 0.543  | 0.090 | +/-0.142 |
| RG25                            | 1.994  | 2.188  | 2.036  | 2.057  | 2.069  | 0.084 | +/-0.133 |
| RG50                            | 4.521  | 4.869  | 4.389  | 4.489  | 4.567  | 0.209 | +/-0.332 |

TABLE J

| SURFACE ANALYSIS SUMMARY        |       |       |       |       |       |       |          |
|---------------------------------|-------|-------|-------|-------|-------|-------|----------|
|                                 | A     | B     | C     | D     | Avg   | STD   | ERR      |
| Example 10A - Warp Direction    |       |       |       |       |       |       |          |
| MIU                             | 0.194 | 0.202 | 0.205 | 0.211 | 0.203 | 0.007 | +/-0.011 |
| MMD                             | 0.027 | 0.027 | 0.029 | 0.024 | 0.027 | 0.002 | +/-0.003 |
| SMD                             | 3.650 | 3.414 | 2.933 | 3.674 | 3.418 | 0.344 | +/-0.547 |
| Example 10A - Filling Direction |       |       |       |       |       |       |          |
| MIU                             | 0.209 | 0.218 | 0.218 | 0.221 | 0.217 | 0.005 | +/-0.008 |
| MMD                             | 0.032 | 0.040 | 0.039 | 0.043 | 0.039 | 0.005 | +/-0.007 |
| SMD                             | 5.891 | 7.340 | 5.596 | 6.440 | 6.317 | 0.767 | +/-1.219 |
| Example 10B - Warp Direction    |       |       |       |       |       |       |          |
| MIU                             | 0.195 | 0.194 | 0.193 | 0.196 | 0.195 | 0.001 | +/-0.002 |
| MMD                             | 0.026 | 0.024 | 0.024 | 0.025 | 0.025 | 0.001 | +/-0.002 |
| SMD                             | 3.730 | 2.776 | 2.465 | 2.846 | 2.954 | 0.543 | +/-0.863 |
| Example 10B - Filling Direction |       |       |       |       |       |       |          |
| MIU                             | 0.202 | 0.205 | 0.203 | 0.204 | 0.204 | 0.001 | +/-0.002 |
| MMD                             | 0.036 | 0.039 | 0.039 | 0.029 | 0.036 | 0.005 | +/-0.008 |
| SMD                             | 7.328 | 7.594 | 7.619 | 6.935 | 7.369 | 0.318 | +/-0.505 |
| Example 10C - Warp Direction    |       |       |       |       |       |       |          |
| MIU                             | 0.192 | 0.197 | 0.194 | 0.196 | 0.195 | 0.002 | +/-0.004 |
| MMD                             | 0.020 | 0.020 | 0.020 | 0.021 | 0.020 | 0.001 | +/-0.001 |
| SMD                             | 2.217 | 2.559 | 2.532 | 2.125 | 2.358 | 0.220 | +/-0.349 |
| Example 10C - Filling Direction |       |       |       |       |       |       |          |

TABLE K

| BENDING ANALYSIS SUMMARY     |       |       |       |       |       |       |          |
|------------------------------|-------|-------|-------|-------|-------|-------|----------|
|                              | A     | B     | C     | D     | Avg   | STD   | ERR      |
| Example 10A - Warp Direction |       |       |       |       |       |       |          |
| B                            | 0.133 | 0.176 | 0.194 | 0.210 | 0.178 | 0.033 | +/-0.053 |

TABLE K-continued

| 30                              | BENDING ANALYSIS SUMMARY |       |       |       |       |       |          |
|---------------------------------|--------------------------|-------|-------|-------|-------|-------|----------|
|                                 | A                        | B     | C     | D     | Avg   | STD   | ERR      |
| 2HB05                           | 0.198                    | 0.225 | 0.235 | 0.276 | 0.234 | 0.032 | +/-0.051 |
| 2HB10                           | 0.213                    | 0.254 | 0.256 | 0.295 | 0.255 | 0.033 | +/-0.053 |
| 2HB15                           | 0.213                    | 0.271 | 0.265 | 0.296 | 0.261 | 0.035 | +/-0.055 |
| RB05                            | 1.492                    | 1.279 | 1.212 | 1.314 | 1.324 | 0.120 | +/-0.190 |
| RB10                            | 1.610                    | 1.443 | 1.319 | 1.405 | 1.444 | 0.122 | +/-0.194 |
| RB15                            | 1.604                    | 1.544 | 1.362 | 1.412 | 1.481 | 0.113 | +/-0.179 |
| Example 10A - Filling Direction |                          |       |       |       |       |       |          |
| B                               | 0.175                    | 0.190 | 0.182 | 0.161 | 0.177 | 0.012 | +/-0.020 |
| 2HB05                           | 0.201                    | 0.215 | 0.205 | 0.178 | 0.200 | 0.016 | +/-0.025 |
| 2HB10                           | 0.218                    | 0.242 | 0.237 | 0.198 | 0.224 | 0.020 | +/-0.032 |
| 2HB15                           | 0.232                    | 0.256 | 0.250 | 0.208 | 0.237 | 0.022 | +/-0.034 |
| RB05                            | 1.147                    | 1.130 | 1.123 | 1.105 | 1.126 | 0.017 | +/-0.028 |
| RB10                            | 1.244                    | 1.272 | 1.302 | 1.234 | 1.263 | 0.031 | +/-0.049 |
| RB15                            | 1.326                    | 1.348 | 1.371 | 1.295 | 1.335 | 0.032 | +/-0.051 |
| Example 10B - Warp Direction    |                          |       |       |       |       |       |          |
| B                               | 0.237                    | 0.210 | 0.221 | 0.239 | 0.227 | 0.014 | +/-0.022 |
| 2HB05                           | 0.264                    | 0.268 | 0.286 | 0.270 | 0.272 | 0.010 | +/-0.015 |
| 2HB10                           | 0.302                    | 0.287 | 0.313 | 0.316 | 0.305 | 0.013 | +/-0.021 |
| 2HB15                           | 0.319                    | 0.300 | 0.319 | 0.329 | 0.317 | 0.012 | +/-0.019 |
| RB05                            | 1.114                    | 1.279 | 1.297 | 1.128 | 1.205 | 0.097 | +/-0.154 |
| RB10                            | 1.277                    | 1.367 | 1.416 | 1.319 | 1.345 | 0.060 | +/-0.096 |
| RB15                            | 1.350                    | 1.428 | 1.445 | 1.375 | 1.400 | 0.044 | +/-0.071 |
| Example 10B - Filling Direction |                          |       |       |       |       |       |          |
| B                               | 0.224                    | 0.243 | 0.224 | 0.202 | 0.223 | 0.017 | +/-0.027 |
| 2HB05                           | 0.264                    | 0.263 | 0.245 | 0.209 | 0.245 | 0.026 | +/-0.041 |
| 2HB10                           | 0.299                    | 0.302 | 0.293 | 0.241 | 0.284 | 0.029 | +/-0.046 |
| 2HB15                           | 0.310                    | 0.316 | 0.301 | 0.255 | 0.296 | 0.028 | +/-0.044 |
| RB05                            | 1.178                    | 1.082 | 1.095 | 1.033 | 1.097 | 0.060 | +/-0.096 |
| RB10                            | 1.333                    | 1.243 | 1.312 | 1.192 | 1.270 | 0.065 | +/-0.103 |
| RB15                            | 1.380                    | 1.304 | 1.348 | 1.262 | 1.324 | 0.051 | +/-0.082 |
| Example 10C - Warp Direction    |                          |       |       |       |       |       |          |
| B                               | 2.529                    | 1.683 | 1.990 | 1.931 | 2.033 | 0.356 | +/-0.566 |
| 2HB05                           | 0.790                    | 0.700 | 0.785 | 0.735 | 0.753 | 0.043 | +/-0.068 |
| 2HB10                           | 0.965                    | 0.824 | 0.944 | 0.869 | 0.901 | 0.066 | +/-0.104 |
| 2HB15                           | 1.013                    | 0.854 | 0.961 | 0.909 | 0.934 | 0.068 | +/-0.109 |
| RB05                            | 0.312                    | 0.416 | 0.394 | 0.381 | 0.376 | 0.045 | +/-0.071 |
| RB10                            | 0.382                    | 0.490 | 0.474 | 0.450 | 0.449 | 0.048 | +/-0.076 |
| RB15                            | 0.400                    | 0.508 | 0.483 | 0.471 | 0.466 | 0.046 | +/-0.074 |

| 60                           | BENDING ANALYSIS SUMMARY |       |       |       |       |       |          |
|------------------------------|--------------------------|-------|-------|-------|-------|-------|----------|
|                              | A                        | B     | C     | D     | Avg   | STD   | ERR      |
| Example 10A - Warp Direction |                          |       |       |       |       |       |          |
| B                            | 0.133                    | 0.176 | 0.194 | 0.210 | 0.178 | 0.033 | +/-0.053 |

TABLE K-continued

| BENDING ANALYSIS SUMMARY        |       |       |       |       |       |       |          |
|---------------------------------|-------|-------|-------|-------|-------|-------|----------|
|                                 | A     | B     | C     | D     | Avg   | STD   | ERR      |
| Example 10C - Filling Direction |       |       |       |       |       |       |          |
|                                 |       |       |       |       |       |       |          |
| B                               | 0.942 | 0.577 | 1.074 | 0.803 | 0.849 | 0.212 | +/-0.338 |
| 2HB05                           | 0.566 | 0.494 | 0.664 | 0.559 | 0.571 | 0.070 | +/-0.111 |
| 2HB10                           | 0.819 | 0.641 | 0.948 | 0.753 | 0.790 | 0.128 | +/-0.204 |
| 2HB15                           | 0.918 | 0.693 | 1.052 | 0.859 | 0.881 | 0.149 | +/-0.237 |
| RB05                            | 0.601 | 0.856 | 0.619 | 0.696 | 0.693 | 0.116 | +/-0.185 |
| RB10                            | 0.870 | 1.112 | 0.883 | 0.937 | 0.951 | 0.112 | +/-0.177 |
| RB15                            | 0.975 | 1.201 | 0.980 | 1.070 | 1.057 | 0.106 | +/-0.168 |

TABLE L

| Kawabata Test Comparison (bottomweight)<br>Example 10 |                                                 |             |             |
|-------------------------------------------------------|-------------------------------------------------|-------------|-------------|
| Kawabata Test                                         | Mean Value                                      |             |             |
|                                                       | Test means significantly different @<br>p = .05 |             |             |
| Group                                                 | Test                                            | Example 10A | Example 10B |
| Shear                                                 | RG50 (Filling)                                  | 4.80        | 5.11        |
| Compression                                           | Comp                                            | 28.82       | 33.64       |
|                                                       | WCprime                                         | 0.08        | 0.10        |
|                                                       | RC                                              | 45.68       | 48.50       |

As indicated, in the Ex. 10 bottomweight samples several tests showed a significant difference between the treatments (see above)

TABLE M

| Example 9B vs. 9C              |        |        |                       |
|--------------------------------|--------|--------|-----------------------|
| Test                           | Ex. 9B | Ex. 9C | Comments              |
| Bending (B):                   |        |        | Higher = More Rigid   |
| Warp                           | 0.096  | 0.161  |                       |
| Filling                        | 0.087  | 0.135  |                       |
| Residual Bending               |        |        | Lower = More Rigid    |
| Curvature (RB05):              |        |        |                       |
| Warp                           | 0.942  | 0.675  |                       |
| Filling                        | 0.918  | 0.823  |                       |
| Coefficient of Friction (MIU): |        |        | Lower = Less Friction |
| Warp                           | 0.221  | 0.201  |                       |
| Filling                        | 0.225  | 0.210  |                       |
| Compression (Den TMax):        |        |        | Lower = Supple Hand   |
| Total                          | 0.441  | 0.501  |                       |
| Mean Shear Stiffness (G):      |        |        | Lower = Supple Hand   |
| Warp                           | 1.233  | 3.241  |                       |
| Filling                        | 1.022  | 3.360  |                       |
| Extensibility (EMT):           |        |        | Higher = More Stretch |
| Warp                           | 2.439  | 1.880  |                       |
| Filling                        | 6.601  | 4.886  |                       |

As indicated, this example showed that the fabric had a unique combination of strength and hand, as evidenced in particular by the Bending (B), Coefficient of Friction (MIU), Filling Tensile Strength, and Filling Tear Strength. In addition, the fabrics of this example had superior colorfastness and flat dry appearance. Preferably, the fabric retains at least about 85%, and more preferably at least about 93% of its initial filling strength, in addition to superior MIU and B values.

TABLE N

| Example 10B vs. 10C |                                |         |         |                       |
|---------------------|--------------------------------|---------|---------|-----------------------|
| 5                   | Test                           | Ex. 10B | Ex. 10C | Comments              |
|                     | Bending (B):                   |         |         | Higher = More Rigid   |
|                     | Warp                           | 0.227   | 2.033   |                       |
|                     | Filling                        | 0.223   | 0.849   |                       |
|                     | Residual Bending               |         |         | Lower = More Rigid    |
| 10                  | Curvature (RB05):              |         |         |                       |
|                     | Warp                           | 1.205   | 0.376   |                       |
|                     | Filling                        | 1.097   | 0.693   |                       |
|                     | Coefficient of Friction (MIU): |         |         | Lower = Less Friction |
|                     | Warp                           | 0.195   | 0.195   |                       |
| 15                  | Filling                        | 0.204   | 0.192   |                       |
|                     | Compression (Den TMax):        |         |         | Lower = Supple Hand   |
|                     | Total                          | 0.451   | 0.464   |                       |
|                     | Mean Shear Stiffness (G):      |         |         | Lower = Supple Hand   |
|                     | Warp                           | 1.707   | 2.573   |                       |
| 20                  | Filling                        | 1.554   | 2.511   |                       |
|                     | Extensibility (EMT):           |         |         | Higher = More Stretch |
|                     | Warp                           | 3.019   | 1.368   |                       |
|                     | Filling                        | 6.325   | 2.489   |                       |

25 Bending is preferably <2 in the warp direction, more preferably <1.5, more preferably <1, even more preferably <0.5, and even more preferably <0.3 in the warp direction. Bending is also preferably <0.8 in the filling direction, more preferably <0.7, more preferably <0.6, <0.5, <0.4, <0.3, or even more preferably <0.25 in the filling direction. In a particularly preferred form of the invention, Bending is low, and the Bending in the warp direction is approximately equal to the Bending in the filling direction.

Also, the RB05 value is preferably  $\geq 0.4$  in the warp direction, more preferably  $\geq 0.5$ , more preferably  $\geq 0.75$ , more preferably  $\geq 1$ , more preferably  $\geq 1.2$ . The RB05 value is also preferably  $\geq 0.75$  in the filling direction, more preferably  $\geq 0.9$ , more preferably  $\geq 1.0$ . RB05 in both warp and fill direction  $\geq 1$ .

35 40 Also, the Mean Shear Stiffness (G) value is preferably  $\leq 2.4$  in the warp direction, more preferably  $\leq 2.2$ , more preferably  $\leq 2$ , more preferably  $\leq 1.8$ . The G value is also more preferably  $\leq 2.4$  in the filling direction, more preferably  $\leq 2.2$ , more preferably  $\leq 2$ , more preferably  $\leq 1.8$ , more preferably  $\leq 1.6$ . G is also preferably  $\leq 2.4$  in both warp and fill directions, more preferably  $\leq 2.2$ , more preferably  $\leq 2$ , more preferably  $\leq 1.8$ .

Also, the % strain at 500 gf/cm value is preferably  $\geq 1.5$  in the warp direction, more preferably  $\geq 2$ , more preferably  $\geq 2.5$ , more preferably  $\geq 3$ . The % strain at 500 gf/cm value is preferably  $\geq 3$  in the filling direction, more preferably  $\geq 4$ , more preferably  $\geq 5$ , more preferably  $\geq 6$ . The % strain at 500 gf/cm value is more preferably  $\geq 3$  in both the warp and filling direction.

55

TABLE O

| Example 10A vs. 10C |                            |         |            |                 |
|---------------------|----------------------------|---------|------------|-----------------|
| 60                  | Construction (Finished)    | Ex. 10A | Ex. 10C    | Industry Specs. |
|                     | Overall Width              | 62.60   | 64.63      |                 |
|                     | Cuttable Width             | 61.35   | 64.00      |                 |
|                     | Ends/Inch                  | 66      | 84         |                 |
|                     | Picks/Inch                 | 48      | 46         |                 |
|                     | Finished Weight (oz/sq yd) | 7.20    | 6.68       |                 |
| 65                  | Warp yarn count - finished | 12/1 OE | 13.6/1 MJS |                 |
|                     | Fill yarn count - finished | 12/1 OE | 13.6/1 MJS |                 |

TABLE O-continued

| <u>Example 10A vs. 10C</u>    |         |         |                 |
|-------------------------------|---------|---------|-----------------|
| Construction (Finished)       | Ex. 10A | Ex. 10C | Industry Specs. |
| Denier - warp                 | 1.20    | 1.18    |                 |
| Twist multiple - warp         | 3.60    | N/A     |                 |
| Denier - fill                 | 1.20    | 1.21    |                 |
| Twist multiple - fill         | 3.60    | N/A     |                 |
| Reed width                    | 72.0    | N/A     |                 |
| <u>Strength</u>               |         |         |                 |
| AR - Tensile - Warp           | 235     | 314     | 150             |
| AR - Tensile - Fill           | 126     | 162     | 100             |
| 10W - Tensile (lbs) Warp      | 230     | 291     |                 |
| 10W - Tensile (lbs) Fill      | 130     | 152     |                 |
| AR - Tear Warp                | 6400    | 6400    | 3400            |
| AR - Tear Fill                | 4739    | 6400    | 3400            |
| 10W - Tear (grams) warp       | 5664    | 6406    |                 |
| 10W - Tear (grams) fill       | 3333    | 4838    |                 |
| Pilling - 10W-60 min          | 4.0     | 1.0     | 3.5             |
| AR - Abrasion (cycles) warp   | 2000    | 2000    | 1000            |
| AR - Abrasion (cycles) fill   | 2000    | 2000    | 1000            |
| AR - Seam slippage (lbs) warp | 40      | 40      | 25              |
| AR - Seam slippage (lbs) fill | 40      | 40      | 20              |
| TOTAL                         | 36      | 37      |                 |
| <u>Wash Performance</u>       |         |         |                 |
| 10 wash shrinkage (%) warp    | 2.8     | 4.5     | 3.0 Max         |
| 10 wash shrinkage (%) fill    | 0.3     | 1.4     | 3.0 Max         |
| 10W - flat dry app.           | 3.5     | 3.0     | 3.5 Min         |
| TOTAL                         | 16      | 12      |                 |
| <u>Comfort</u>                |         |         |                 |
| Moisture transport (sec)      | 1.0     | 1.0     |                 |
| Drape test value              | 129     | 438     | Lower = Better  |
| TOTAL                         | 43      | 28      |                 |

AR = As received

TABLE P

Example 9A vs. 9B vs. 9C

| Construction (Finished)       | Ex. 9A  | Ex. 9B  | Ex. 9C | Industry Specs. |
|-------------------------------|---------|---------|--------|-----------------|
| Overall Width                 | 64.63   | 63.25   | 61.00  |                 |
| Cuttable Width                | 63.38   | 62.00   | 60.50  |                 |
| Ends/Inch                     | 82      | 81      | 84     |                 |
| Picks/Inch                    | 47      | 48      | 72     |                 |
| Finished Weight (oz/sq yd)    | 4.40    | 4.48    | 4.56   | 4.25-4.50       |
| Warp yarn count - finished    | 19/1 OE | 19/1 OE | 25.5/1 | MJS             |
| Fill yarn count - finished    | 26/1 OE | 26/1 OE | 24.8/1 | MJS             |
| Denier - warp                 | 1.20    | 1.20    | 1.27   |                 |
| Twist multiple - warp         | 3.60    | 3.60    | N/A    |                 |
| Denier - fill                 | 1.20    | 1.20    | 1.26   |                 |
| Twist multiple - fill         | 3.50    | 3.50    | N/A    |                 |
| Reed width                    | 72.0    | 72.0    | N/A    |                 |
| <u>Strength</u>               |         |         |        |                 |
| AR - Tensile - Warp           | 162     | 162     | 171    | 60              |
| AR - Tensile - Fill           | 56      | 80      | 137    | 50              |
| 10W - Tensile (lbs) Warp      | 163     | 161     | 167    |                 |
| 10W - Tensile (lbs) Fill      | 57      | 85      | 138    |                 |
| AR - Tear Warp                | 3333    | 3629    | 2778   | 1135            |
| AR - Tear Fill                | 1750    | 3512    | 2214   | 1135            |
| 10W - Tear (grams) warp       | 2716    | 2355    | 2042   |                 |
| 10W - Tear (grams) fill       | 1275    | 1529    | 1741   |                 |
| Pilling - 10W-60 min          | 4.2     | 4.0     | 1.0    | 3.5             |
| AR - Abrasion (cycles) warp   | 2000    | 2000    | 2000   | 1000            |
| AR - Abrasion (cycles) fill   | 2000    | 2000    | 2000   | 1000            |
| AR - Seam slippage (lbs) warp | 37      | 40      | 40     | 25              |
| AR - Seam slippage (lbs) fill | 40      | 40      | 40     | 20              |

TABLE P-continued

| <u>Example 9A vs. 9B vs. 9C</u> |        |        |        |                 |
|---------------------------------|--------|--------|--------|-----------------|
| Construction (Finished)         | Ex. 9A | Ex. 9B | Ex. 9C | Industry Specs. |
| TOTAL                           | 34     | —      | 36     |                 |
| <u>Wash Performance</u>         |        |        |        |                 |
| 10 wash shrinkage (%) warp      | 1.6    | 1.7    | 3.5    |                 |
| 10 wash shrinkage (%) fill      | 0.0    | 1.0+   | 1.0    |                 |
| 10W - flat dry app.             | 3.3    | 3.5    | 2.0    | 3.0 Min         |
| TOTAL                           | 22     | —      | 13     |                 |
| <u>Comfort</u>                  |        |        |        |                 |
| Moisture transport (sec)        | 2.0    | 2.0    | 2.0    |                 |
| Drape test value                | 94     | 97     | 555    | Lower = Better  |
| TOTAL                           | 43     | —      | 28     |                 |

AR = As received

20 As illustrated by the test data, the 100% spun polyester shirting of the instant invention had superior hand to conventional polyester cotton shirting materials, had much improved color wash down, had quicker dry time (which enables it to utilize a shortened dry cycle or lower dry temperatures and less energy output), no directionality on dyed shades, improved tensile performance, superior initial warp tear strength, superior initial filling tear strength, and higher initial warp tensile strength. In addition, the 100% polyester product made by the process of the instant invention had a superior characteristics relative to a conventionally sanded 100% polyester fabric (i.e. Ex 9B vs. 9C) as follows: substantially improved pilling, substantially better wash shrinkage when subjected to industrial washes, improved flat dry appearance following industrial washing, and no directionality.

30 More specifically, for fabrics of the variety described in Ex. 9, the fabrics preferably have a WT of >0.3, more preferably >0.4, even more preferably >0.5, >0.6, >0.7, and/or greater than 0.8, but preferably less than 0.9.

40 In addition, the 100% polyester product of the invention had the following benefits as compared with commercially available 100% polyester fabrics of similar weight designed for the same types of markets: substantially better pilling (tested according the Random Tumble Method), wash shrinkage after 10 industrial washings at 165°, improved flat dry appearance after 10 industrial washes at 165°, no directionality, and significantly better drape and hand.

45 It is not intended that the scope of the invention be limited to the specific embodiments described herein, rather, it is intended that the scope of the invention be defined by the appended claims and their equivalents.

50 What is claimed is:

55 1. A woven fabric comprising warp and filling yarns, said woven fabric comprising synthetic fibers, wherein said woven fabric includes a plurality of surface fibers, and at least a plurality of said surface fibers comprise a plurality of cuts at random locations on said individual fibers and a plurality of cut fiber ends defining a uniformly short pile, with at least some of said cut fiber ends being from the warp yarns, and wherein said cuts serve as stress risers on the individual fibers, allowing the fibers to break off during bending, and wherein said uniformly short pile is produced by abrasion of a greige fabric wherein at least the surface fibers of said greige fabric are encapsulated in a coating matrix and wherein abrasion of said greige fabric results in nicks on the surface fibers.

**31**

2. A woven fabric comprising warp and filling yarns, said woven fabric containing spun yams incorporating at least 65% polyester fibers, wherein said fabric has a weight of about 4.5 oz/sq yd and a consistently short pile defined by cut ends of fibers forming the woven fabric, wherein said fabric has a Kawabata System Coefficient of Friction MIU value of at least 0.2 and a filling tear strength of about 2500 lbs or greater, and wherein said uniformly short pile is produced by abrasion of a greige fabric wherein at least the surface fibers of said greige fabric are encapsulated in a coating matrix and wherein abrasion of said greige fabric results in nicks on the surface fibers.

3. A woven fabric comprising a plurality of warp and filling yarns, said woven fabric having an abraded surface defining a consistent short pile, and surface fibers having a plurality of cuts at random locations on individual fibers, wherein said fabric has a Kawabata System Coefficient of Friction MIU of about 0.2 or greater, wherein said fabric has a retained filling strength following abrasion of at least about 85% of its filling strength prior to abrasion, and wherein said uniformly short pile is produced by abrasion of a greige fabric wherein at least the surface fibers of said greige fabric are encapsulated in a coating matrix and wherein abrasion of said greige fabric results in nicks on the surface fibers.

4. A woven fabric according to claim 1, wherein said cuts and cut fiber ends define an abraded surface, and wherein said fabric has a filling strength in a filling direction following abrasion of at least about 85% of its filling strength prior to abrasion.

5. A woven fabric comprising warp and filling yarns, said woven fabric comprising synthetic fibers, wherein said woven fabric includes a plurality of surface fibers, and at least a plurality of said surface fibers comprise a plurality of cuts at random locations on said individual fibers and a

**32**

plurality of cut fiber ends defining a uniformly short pile, with at least some of said cut fiber ends being from the warp yams, and wherein said cuts serve as stress risers on the individual fibers, allowing the fibers to break off during bending, wherein said cuts and cut fiber ends are formed by immobilizing fibers while subjecting them to abrasion, sanding or napping.

6. A woven fabric according to claim 2, wherein said cuts and cut fiber ends define an abraded surface, and wherein said fabric has a filling strength in a filling direction following abrasion of at least about 85% of its filling strength prior to abrasion.

7. A woven fabric comprising warp and filling yarns, said woven fabric containing spun yams incorporating at least 65% polyester fibers, wherein said fabric has a weight of about 4.5 oz/sq yd and a consistently short pile defined by cut ends of fibers forming the woven fabric, wherein said fabric has a Kawabata System Coefficient of Friction MIU value of at least 0.2 and a filling tear strength of about 2500 lbs or greater, wherein said cuts and cut fiber ends are formed by immobilizing fibers while subjecting them to abrasion, sanding or napping.

8. A woven fabric comprising a plurality of warp and filling yams, said woven fabric having an abraded surface defining a consistent short pile, and surface fibers having a plurality of cuts at random locations on individual fibers, wherein said fabric has a Kawabata System Coefficient of Friction MIU of about 0.2 or greater, wherein said fabric has a retained filling strength following abrasion of at least about 85% of its filling strength prior to abrasion, wherein said cuts and short pile ends are formed by immobilizing fibers while subjecting them to abrasion, sanding or napping.

\* \* \* \* \*